



**Related U.S. Application Data**

|                                                                                                    |                   |         |                                 |
|----------------------------------------------------------------------------------------------------|-------------------|---------|---------------------------------|
| continuation-in-part of application No. 12/852,147, filed on Aug. 6, 2010, now Pat. No. 8,802,605. | 5,863,999 A       | 1/1999  | Kinker                          |
| (60) Provisional application No. 61/232,060, filed on Aug. 7, 2009.                                | 5,955,405 A       | 9/1999  | Liesen                          |
|                                                                                                    | 5,969,068 A       | 10/1999 | Bryant                          |
|                                                                                                    | 6,034,040 A       | 3/2000  | Ozbalik                         |
|                                                                                                    | 6,063,146 A       | 5/2000  | Miller                          |
|                                                                                                    | 6,133,210 A       | 10/2000 | Tipton                          |
|                                                                                                    | 6,140,431 A       | 10/2000 | Kinker                          |
|                                                                                                    | 6,255,261 B1      | 7/2001  | Liesen                          |
|                                                                                                    | 6,290,869 B1      | 9/2001  | Sorensen                        |
|                                                                                                    | 6,291,409 B1 *    | 9/2001  | Kodali et al. .... 508/491      |
| (51) <b>Int. Cl.</b>                                                                               | 6,294,628 B1      | 9/2001  | Bryant                          |
| <i>C10M 145/04</i>                                                                                 | 6,323,164 B1      | 11/2001 | Liesen                          |
| <i>C10M 141/06</i>                                                                                 | 6,326,514 B1      | 12/2001 | Klug                            |
| <i>C10M 129/93</i>                                                                                 | 6,348,554 B1      | 2/2002  | Roos                            |
| <i>C10M 129/10</i>                                                                                 | 6,391,996 B1      | 5/2002  | Scherer                         |
| <i>C10M 129/40</i>                                                                                 | 6,403,745 B1      | 6/2002  | Scherer                         |
| <i>C10M 133/44</i>                                                                                 | 6,403,746 B1      | 6/2002  | Roos                            |
|                                                                                                    | 6,458,749 B2      | 10/2002 | Kinker                          |
|                                                                                                    | 6,511,946 B1      | 1/2003  | Theis                           |
|                                                                                                    | 6,525,006 B2      | 2/2003  | Yoneta                          |
|                                                                                                    | 6,569,969 B2      | 5/2003  | Charmot                         |
|                                                                                                    | 6,586,375 B1      | 7/2003  | Gahagan                         |
|                                                                                                    | 6,610,801 B1      | 8/2003  | Scherer                         |
|                                                                                                    | 6,610,802 B2      | 8/2003  | Roos                            |
|                                                                                                    | 6,627,584 B2      | 9/2003  | Ozbalik                         |
|                                                                                                    | 6,712,991 B2      | 3/2004  | Gore                            |
|                                                                                                    | 6,780,824 B2      | 8/2004  | Oelscher                        |
|                                                                                                    | 6,787,663 B2      | 9/2004  | Adams                           |
|                                                                                                    | 6,803,050 B2      | 10/2004 | Denzer                          |
|                                                                                                    | 6,881,780 B2      | 4/2005  | Bryant                          |
|                                                                                                    | 7,008,561 B2      | 3/2006  | Dahlmann                        |
|                                                                                                    | 7,189,682 B2      | 3/2007  | Gapinski                        |
|                                                                                                    | 7,208,118 B2      | 4/2007  | Leinweber                       |
|                                                                                                    | 7,214,276 B2      | 5/2007  | Dahlmann                        |
|                                                                                                    | 7,429,555 B2      | 9/2008  | Scherer                         |
|                                                                                                    | 7,470,381 B2      | 12/2008 | Placek                          |
|                                                                                                    | 7,553,673 B2      | 6/2009  | Kinker                          |
|                                                                                                    | 7,560,420 B2      | 7/2009  | Kinker                          |
|                                                                                                    | 7,615,522 B2      | 11/2009 | Camenzind                       |
|                                                                                                    | 7,645,842 B2      | 1/2010  | Acker                           |
|                                                                                                    | 7,648,950 B2      | 1/2010  | Placek                          |
|                                                                                                    | 7,851,420 B2      | 12/2010 | Theunissen                      |
|                                                                                                    | 7,875,581 B2      | 1/2011  | Chiba                           |
|                                                                                                    | 8,343,905 B2      | 1/2013  | Gutierrez                       |
|                                                                                                    | 2003/0194388 A1   | 10/2003 | Dahlmann                        |
|                                                                                                    | 2004/0014611 A1 * | 1/2004  | Li .... 508/214                 |
|                                                                                                    | 2004/0014879 A1   | 1/2004  | Denzer                          |
|                                                                                                    | 2004/0235680 A1   | 11/2004 | Lawrence                        |
|                                                                                                    | 2005/0197261 A1   | 9/2005  | Leinweber et al.                |
|                                                                                                    | 2005/0262643 A1   | 12/2005 | Nogues Lopez                    |
|                                                                                                    | 2005/0288191 A1   | 12/2005 | Lawrence                        |
|                                                                                                    | 2007/0184202 A1   | 8/2007  | Rochfort                        |
|                                                                                                    | 2007/0197407 A1   | 8/2007  | Bardasz                         |
|                                                                                                    | 2008/0076687 A1   | 3/2008  | Habeb                           |
|                                                                                                    | 2009/0017243 A1 * | 1/2009  | Person Hei et al. .... 428/35.7 |
|                                                                                                    | 2010/0009879 A1 * | 1/2010  | Theyssen et al. .... 508/431    |
|                                                                                                    | 2010/0081716 A1   | 4/2010  | Matsunaga                       |
|                                                                                                    | 2010/0130392 A1   | 5/2010  | Theyssen                        |
|                                                                                                    | 2010/0286009 A1   | 11/2010 | Vierbaum                        |
|                                                                                                    | 2011/0034359 A1   | 2/2011  | Rabbat                          |

**References Cited**

## U.S. PATENT DOCUMENTS

|             |         |              |    |             |         |
|-------------|---------|--------------|----|-------------|---------|
| 2,745,857 A | 5/1956  | Britton      | CN | 101437931 A | 5/2009  |
| 2,801,972 A | 8/1957  | Bartlett     | DE | 2418444 A1  | 10/1975 |
| 2,803,646 A | 8/1957  | Bell         | DE | 4244536 A1  | 7/1994  |
| 3,625,893 A | 12/1971 | Brook        | DE | 19730085 A1 | 1/1999  |
| 3,755,176 A | 8/1973  | Kinney       | DE | 19747895 A1 | 5/1999  |
| 3,791,971 A | 2/1974  | Lowe         | DE | 19833894 A1 | 3/2000  |
| 3,828,086 A | 8/1974  | Kenney       | DE | 19956237 A1 | 5/2001  |
| 3,856,688 A | 12/1974 | Kenney       | EP | 0399751 A3  | 11/1990 |
| 3,890,381 A | 6/1975  | Kiyoura      | EP | 0566956 A1  | 10/1993 |
| 3,956,382 A | 5/1976  | Krause       | EP | 0430602 B1  | 9/1995  |
| 3,992,443 A | 11/1976 | Springmann   | EP | 1652909 A1  | 5/2006  |
| 4,088,590 A | 5/1978  | Knoblauch    | EP | 2050806 A1  | 4/2009  |
| 4,098,818 A | 7/1978  | Krummel      | EP | 20425887 A1 | 4/2009  |
| 4,214,101 A | 7/1980  | Miya         | JP | 2097592 A   | 4/1990  |
| 4,265,774 A | 5/1981  | Langdon      | JP | 2097593 A   | 4/1990  |
| 4,579,672 A | 4/1986  | Brecker      | JP | 08333592    | 12/1996 |
| 4,625,057 A | 11/1986 | Springmann   |    |             |         |
| 4,713,487 A | 12/1987 | Sekine       |    |             |         |
| 4,719,052 A | 1/1988  | Ohsaka       |    |             |         |
| 4,784,781 A | 11/1988 | Denis        |    |             |         |
| 4,898,687 A | 2/1990  | Parker       |    |             |         |
| 4,954,273 A | 9/1990  | Denis        |    |             |         |
| 4,976,893 A | 12/1990 | Leupold      |    |             |         |
| 4,978,785 A | 12/1990 | Sanderson    |    |             |         |
| 5,013,482 A | 5/1991  | O'Neil       |    |             |         |
| 5,223,642 A | 6/1993  | Schonwalder  |    |             |         |
| 5,230,823 A | 7/1993  | Wise         |    |             |         |
| 5,233,087 A | 8/1993  | Cripe        |    |             |         |
| 5,250,203 A | 10/1993 | Denis        |    |             |         |
| 5,263,308 A | 11/1993 | Lee          |    |             |         |
| 5,275,809 A | 1/1994  | Chen         |    |             |         |
| 5,282,987 A | 2/1994  | Balzer       |    |             |         |
| 5,292,940 A | 3/1994  | Carduck      |    |             |         |
| 5,296,218 A | 3/1994  | Chen         |    |             |         |
| 5,368,761 A | 11/1994 | Gore         |    |             |         |
| 5,374,366 A | 12/1994 | Nakahara     |    |             |         |
| 5,412,049 A | 5/1995  | Argyropoulos |    |             |         |
| 5,440,000 A | 8/1995  | Shirodkar    |    |             |         |
| 5,463,114 A | 10/1995 | Noack        |    |             |         |
| 5,490,950 A | 2/1996  | Smid         |    |             |         |
| 5,516,440 A | 5/1996  | Dasai        |    |             |         |
| 5,576,470 A | 11/1996 | Tuller       |    |             |         |
| 5,597,871 A | 1/1997  | Auschra      |    |             |         |
| 5,609,862 A | 3/1997  | Chen         |    |             |         |
| 5,773,505 A | 6/1998  | Pennewiss    |    |             |         |
| 5,843,874 A | 12/1998 | Macpherson   |    |             |         |

## FOREIGN PATENT DOCUMENTS

(56)

## References Cited

## FOREIGN PATENT DOCUMENTS

|    |                  |         |
|----|------------------|---------|
| JP | 09040982         | 2/1997  |
| JP | 09040990         | 2/1997  |
| JP | 11199881         | 7/1999  |
| JP | 2001335696       | 12/2001 |
| JP | 2002212007       | 7/2002  |
| JP | 2002275483 A     | 9/2002  |
| JP | 2005247850 A     | 9/2005  |
| JP | 2008031149       | 2/2008  |
| JP | 2008106253       | 5/2008  |
| JP | 2009096997       | 5/2009  |
| JP | 2009197338       | 9/2009  |
| KR | 10-1999-021224 A | 3/1999  |
| PL | 314357 A1        | 11/1996 |
| PL | 182003 B1        | 10/2001 |
| WO | 9856881 A1       | 12/1998 |
| WO | 2004037960 A1    | 5/2004  |
| WO | 2008073951 A1    | 6/2008  |
| ZA | 9809884 A        | 4/1999  |

## OTHER PUBLICATIONS

English language abstract and translation for DE 19956237 extracted from the espacenet.com database, 16 pages, (2001).

English language abstract and translation for JP 2009-197338 extracted from the PAJ database, 43 pages, (2009).

English language abstract for DE 4244536 extracted from the espacenet.com database on Aug. 17, 2011, 7 pages.

English language abstract for DE 19730085 extracted from the espacenet.com database on Aug. 18, 2011, 5 pages.

English language abstract for DE 19747895 extracted from the espacenet.com database on Aug. 17, 2011, 27 pages.

English language abstract for EP 0566956 extracted from the espacenet.com database on Aug. 17, 2011, 9 pages.

English language abstract for EP 2050806 extracted from the espacenet.com database on Aug. 17, 2011, 11 pages.

English language abstract and translation for JP 08333592 extracted from the PAJ database on Aug. 17, 2011, 18 pages.

English language abstract and translation for JP 09040982 extracted from the PAJ database on Aug. 17, 2011, 25 pages.

English language abstract and translation for JP 09040990 extracted from the PAJ database on Aug. 17, 2011, 25 pages.

English language abstract and translation for 11199881 extracted from the PAJ database on Aug. 17, 2011, 33 pages.

English language abstract and translation for JP 2001335696 extracted from the Paj database on Aug. 17, 2011, 23 pages.

English language abstract and translation for JP 2002212007 extracted from the PAJ database on Aug. 17, 2011, 26 pages.

English language abstract and translation for JP 2008106253 extracted from the PAJ database on Aug. 17, 2011, 49 pages.

English language abstract and translation for JP 2008031149 extracted from the PAJ database on Aug. 17, 2011, 150 pages.

English language abstract and translation for JP 2009096997 extracted from the PAJ database on Aug. 17, 2011, 138 pages.

English language abstract and translation for JP 2009197338 extracted from the PAJ database on Aug. 17, 2011, 56 pages.

English language abstract for PL 314357. Original document not available. However, see foreign language equivalent PL 182003, 10 pages, (2001).

Zhao et al., "Oxidation of Primary Alcohols to Carboxylic Acids with Sodium Chlorite Catalyzed by Tempo and Bleach: 4-Methoxyphenylacetic Acid," *Organic Synthesis*, 2005, vol. 81, p. 195-203.

English language abstract for EP 1652909 extracted from the espacenetcom database on Jul. 31, 2012, 14 pages.

International Search Report for Application No. PCT/US2012/036327 dated Jul. 11, 2012, 3 pages.

English language abstract for JP 2097593 abstractad from aspacanat.com database, dated Dec. 14, 2010, 6 pages.

English language abstract for JP 2097592 abstractad from aspacanat.com database, dated Dec. 14, 2010, 6 pages.

English language abstract for JP 2002275483 abstractad from aspacanat.com database, dated Dec. 14, 2010, 8 pages.

"Alcohols, Aliphatic" Falbe, J., Bahrmann, H., Lipps, W. and Mayer, D. 2000. Alcohols, Aliphatic. *Ullmann's Encyclopedia of Industrial Chemistry*, 27 pages.

Technical Paper, "New Generation of Ashless Top Tier Hydraulic Fluids", Lubrication Engineering, Clark, at al., Apr. 2000, 10 pages.

"Fatty Alcohols", Nowack, at al., *Ullmann's Encyclopedia of Industrial Chemistry*, 2006, 26 pages.

PCT International Search Report, Application No. PCT/US2010/044747, dated Nov. 19, 2010, 3 pages.

Appendix E—"API Base Oil Interchangeability Guidelines for Passenger Car Motor Oils and Diesel Engine Oils" API 1509, Engine Oil Licensing and Certification System, 16th Edition, Apr. 2007, 26 pages.

English language abstract for DE 19956237 extracted from espacenet.com database, dated Jan. 5, 2011, 9 pages.

English language abstract for DE 19833894 extracted from espacenet.com database, dated Jan. 5, 2011, 7 pages.

Article; Betty Burke, et al. *Journal of ASTM International "Contamination of Power Generationtont Lubricants"*, vol. 4, No. 10, Nov. 2007, available 333 online at [www.sstem.org](http://www.sstem.org), 7 pages.

Article; D. Clark, et al., "New Generation of Ashless Top Tier Hydraulic Fluids/North America", not dated, printed off the website on Jan. 14, 2011, 10 pages.

English equivalent for DE 24 18 444 extracted from espacenet.com on Jan. 24, 2011, 23 pages.

English language abstract for CN 101437931 extracted from espacenet.com database on Jul. 24, 2013, 18 pages.

No English language abstract available for DE 2418444. However, see English language equivalent U.S. Pat. No. 3992443. Extracted from the spacenet.com database on Aug. 18, 2011, 23 pages.

English language abstract and machine-assisted English translation of Claims for KR 10-1999-021224 extracted from KIPO database on Dec. 29, 2015, 3 pages.

\* cited by examiner



Figure 1



Figure 2

## LUBRICANT COMPOSITION

## RELATED APPLICATIONS

This application is a CON of Ser. No. 12/852,147 filed Aug. 6, 2010, now U.S. Pat. No. 8,802,605 which claims benefit of 61/232,060 filed Aug. 7, 2009 and a CON of Ser. No. 13/182,116 filed Jul. 13, 2011, now U.S. Pat. No. 8,802,606 which is a CIP of Ser. No. 12/852,147 which claims benefit of 61/232,060 Aug. 7, 2009.

## FIELD OF THE DISCLOSURE

The present disclosure generally relates to a lubricant composition that is substantially free of water and includes an alkylethercarboxylic acid corrosion inhibitor, a base oil, and an antioxidant. More specifically, the alkylethercarboxylic acid corrosion inhibitor includes an alkyl chain having 6 to 18 carbon atoms.

## DESCRIPTION OF THE RELATED ART

Lubricant compositions are generally well known in the art and are broadly categorized as oil or water based compositions, i.e., compositions that include large weight percentages of non-polar compounds (such as (base) oils) or large weight percentages of water, respectively. Lubricant compositions are typically further categorized as engine oils, driveline system oils, gear oils, greases, automatic and manual transmission fluids and oils, hydraulic oils, industrial gear oils, turbine oils, rust and oxidation (R&O) inhibited oils, compressor oils, or paper machine oils, etc. Each of these compositions has particular specifications and design requirements and most are designed to minimize corrosion and wear, to resist thermal and physical breakdown, and to be able to minimize the effects of common contaminants such as oxidizing compounds and metal fragments.

Additives such as corrosion inhibitors and antiwear additives can be utilized to improve corrosion and wear resistance of the composition, respectively. However, it is well known in the art that corrosion inhibitors act antagonistically to antiwear additives to reduce the effectiveness of antiwear additives. For this reason, trade-offs are made when formulating compositions to balance corrosion and wear resistance.

In addition, many oil based lubricant compositions, such as those that include nonylphenolic corrosion inhibitors, have low compatibility with calcium ions and water present in many applications and tend to physically break down, i.e., emulsify and/or phase combine with the water. As a result, decreased amounts of such corrosion inhibitors are used to reduce emulsification and to promote phase separation such that the lubricant compositions can remain intact and separate from water. However, by decreasing the amounts of corrosion inhibitors used, the protection provided by the lubricant compositions against corrosion also decreases. This is commercially and practically undesirable. Accordingly, there remains an opportunity to develop an improved lubricant composition.

## SUMMARY OF THE DISCLOSURE AND ADVANTAGES

The instant disclosure provides a lubricant composition that is substantially free of water and includes a base oil present in an amount of greater than 85 parts by weight per 100 parts by weight of the lubricant composition, includes an antioxidant, and includes one or more alkylethercarboxylic

acid corrosion inhibitor(s) present in an amount of from 0.01 to 1 weight percent based on a total weight of the lubricant composition. The one or more alkylethercarboxylic acid corrosion inhibitor(s) have the formula;



wherein R is a straight or branched chain C<sub>6</sub>-C<sub>18</sub> alkyl group and n is a number of from 0 to 5.

The one or more alkylethercarboxylic acid corrosion inhibitor(s) tend to be effective at low concentrations and tend to exhibit excellent demulsibility and calcium compatibility in a variety of lubricant compositions. In addition, the one or more alkylethercarboxylic acid corrosion inhibitor(s) reduce corrosion of steel articles steel while simultaneously minimizing negative interactions with (e.g. antagonism of) anti-wear additives and detergents, when utilized.

In various embodiments, the lubricant composition also includes an ashless antiwear additive including phosphorous and has improved four-ball antiwear properties. In such embodiments, the one or more alkylethercarboxylic acid corrosion inhibitor(s) unexpectedly enhances the effect of the antiwear additives relative to the four-ball antiwear properties. At the same time, the corrosion inhibitor allows the composition to have excellent corrosion resistance properties when applied to the metal. This combination of excellent antiwear and corrosion resistance properties unexpectedly contradicts traditional wisdom.

## BRIEF DESCRIPTION OF THE SEVERAL VIEWS OF THE DRAWINGS

Other advantages of the present disclosure will be readily appreciated, as the same becomes better understood by reference to the following detailed description when considered in connection with the accompanying drawings wherein:

FIG. 1 is a bar graph that shows the average wear scars (mm) measured in a Four-Ball Antiwear Test (ASTM D4172) as a function of Examples 1(A-C)-10(A-C) from the second set of Examples; and

FIG. 2 is a line graph that shows the average wear scars (mm) measured in a Four-Ball Antiwear Test (ASTM D4172) as a function of the treat rate of various comparative corrosion inhibitors and a corrosion inhibitor from the second set of Examples.

## DETAILED DESCRIPTION OF THE DISCLOSURE

The present disclosure provides a lubricant composition. The lubricant composition may be further defined as ash-containing or ash-less, according to ASTM D 874 and known in the art. Typically, the terminology "ash-less" refers to the absence of (significant) amounts of metals such as sodium, potassium, calcium, and the like. Of course, it is to be understood that the lubricant composition is not particularly limited to being defined as either ash-containing or ash-less.

In various embodiments, the lubricant composition can be further described as a fully formulated lubricant or alternatively as an engine oil. In one embodiment, the terminology "fully formulated lubricant" refers to a total final composition that is a final commercial oil. This final commercial oil may include, for instance, detergents, dispersants, antioxidants,

antifoam additives, pour point depressants, viscosity index improvers, anti-wear additives, friction modifiers, and other customary additives. In the art, engine oils may be referred to as including a base oil as described below and performance additives. The lubricant composition may be as described in U.S. Ser. No. 61/232,060, filed on Aug. 7, 2009, the disclosure of which is expressly incorporated herein by reference in its entirety in one or more non-limiting embodiments.

The lubricant composition (hereinafter referred to as "composition") can include a base oil in addition and one or more alkylethercarboxylic acid corrosion inhibitor(s), each of which are described in greater detail below. Alternatively, the composition can include a base oil, one or more alkylethercarboxylic acid corrosion inhibitor(s), and an ashless antiwear additive including phosphorous, each of which are described in greater detail below. In various embodiments, the composition may consist essentially of the base oil, the one or more alkylethercarboxylic acid corrosion inhibitor(s), and optionally the ashless antiwear additive including phosphorous. In such an embodiment, the composition is typically free of (or includes less than 10 wt %, 5 wt %, 1 wt %, 0.5 wt %, or 0.1 wt %) ashed antiwear additives, additional corrosion inhibitors, etc. Alternatively, the composition may consist of the base oil, the one or more alkylethercarboxylic acid corrosion inhibitor(s), and optionally the ashless antiwear additive including phosphorous.

#### Base Oil:

The base oil is not particularly limited and may be further defined as including one or more oils of lubricating viscosity such as natural and synthetic lubricating or base oils and mixtures thereof. In one embodiment, the base oil is further defined as a lubricant. In another embodiment, the base oil is further defined as an oil of lubricating viscosity. In still another embodiment, the base oil is further defined as a crank-case lubricating oil for spark-ignited and compression ignited internal combustion engines, including automobile and truck engines, two-cycle engines, aviation piston engines, and marine and railroad diesel engines. Alternatively, the base oil can be further defined as an oil to be used in gas engines, stationary power engines, and turbines. The base oil may be further defined as a heavy or light duty engine oil. In one embodiment, the base oil is further defined as a heavy duty diesel engine oil. Alternatively, the base oil may be described as an oil of lubricating viscosity or lubricating oil, for instance as disclosed in U.S. Pat. No. 6,787,663 and U.S. 2007/0197407, each of which is expressly incorporated herein by reference in one or more non-limiting embodiments. Alternatively, the base oil may be used in or as an engine oil, driveline system oil, gear oil, grease, automatic and manual transmission fluid or oil, hydraulic oil, industrial gear oil, turbine oil, rust and oxidation (R&O) inhibited oil, compressor oil, or paper machine oil, etc. It is also contemplated that the base oil may be as described in U.S. Ser. No. 61/232,060, filed on Aug. 7, 2009, the disclosure of which is expressly incorporated herein by reference in its entirety in one or more non-limiting embodiments.

The base oil may be further defined as a base stock oil. Alternatively, the base oil may be further defined as a component that is produced by a single manufacturer to the same specifications (independent of feed source or manufacturer's location) that meets the same manufacturer's specification and that is identified by a unique formula, product identification number, or both. The base oil may be manufactured or derived using a variety of different processes including but not limited to distillation, solvent refining, hydrogen processing, oligomerization, esterification, and re-refining. Re-refined stock is typically substantially free from materials introduced through manufacturing, contamination, or previous use. In one embodiment, the base oil is further defined as a base stock slate, as is known in the art.

Alternatively, the base oil may be derived from hydrocracking, hydrogenation, hydrofinishing, refined and re-refined oils or mixtures thereof or may include one or more such oils. In one embodiment, the base oil is further defined as an oil of lubricating viscosity such as a natural or synthetic oil and/or combinations thereof. Natural oils include, but are not limited to, animal oils and vegetable oils (e.g., castor oil, lard oil) as well as liquid petroleum oils and solvent-treated or acid-treated mineral lubricating oils such as paraffinic, naphthenic or mixed paraffinic-naphthenic oils.

In various other embodiments, the base oil may be further defined as an oil derived from coal or shale. Non-limiting examples of suitable oils include hydrocarbon oils such as polymerized and interpolymerized olefins (e.g., polybutylenes, polypropylenes, propylene-isobutylene copolymers, poly(1-hexenes), poly(1-octenes), poly(1-decenes), and mixtures thereof; alkylbenzenes (e.g., dodecylbenzenes, tetradecylbenzenes, dinonylbenzenes, and di(2-ethylhexyl)-benzenes); polyphenyls (e.g., biphenyls, terphenyls, and alkylated polyphenyls), alkylated diphenyl ethers and alkylated diphenyl sulfides and the derivatives, analogs, and homologs thereof.

In still other embodiments, the base oil may be further defined as a synthetic oil which may include one or more alkylene oxide polymers and interpolymers and derivatives thereof wherein terminal hydroxyl groups are modified by esterification, etherification, or similar reactions. Typically, these synthetic oils are prepared through polymerization of ethylene oxide or propylene oxide to form polyoxyalkylene polymers which can be further reacted to form the oils. For example, alkyl and aryl ethers of these polyoxyalkylene polymers (e.g., methylpolyisopropylene glycol ether having an average molecular weight of 1,000; diphenyl ether of polyethylene glycol having a molecular weight of 500-1,000; and diethyl ether of polypropylene glycol having a molecular weight of 1,000-1,500) and/or mono- and polycarboxylic esters thereof (e.g. acetic acid esters, mixed C<sub>3</sub>-C<sub>8</sub> fatty acid esters, or the C<sub>13</sub> oxo acid diester of tetraethylene glycol) may also be utilized.

In even further embodiments, the base oil may include esters of dicarboxylic acids (e.g., phthalic acid, succinic acid, alkyl succinic acids and alkenyl succinic acids, maleic acid, azelaic acid, suberic acid, sebacic acid, fumaric acid, adipic acid, linoleic acid dimer, malonic acid, alkyl malonic acids, and alkenyl malonic acids) with a variety of alcohols (e.g., butyl alcohol, hexyl alcohol, dodecyl alcohol, 2-ethylhexyl alcohol, ethylene glycol, diethylene glycol monoether, and propylene glycol). Specific examples of these esters include, but are not limited to, dibutyl adipate, di(2-ethylhexyl) sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, the complex ester formed by reacting one mole of sebacic acid with two moles of tetraethylene glycol and two moles of 2-ethylhexanoic acid, and combinations thereof. Esters useful as the base oil or as included in the base oil also include those formed from C<sub>5</sub> to C<sub>12</sub> monocarboxylic acids and polyols and polyol ethers such as neopentyl glycol, trimethylolpropane, pentaerythritol, dipentaerythritol, and tri-pentaerythritol.

The base oil may be alternatively described as a refined and/or re-refined oil, or combinations thereof. Unrefined oils are typically obtained from a natural or synthetic source without further purification treatment. For example, a shale oil obtained directly from retorting operations, a petroleum oil obtained directly from distillation, or an ester oil obtained directly from an esterification process and used without further treatment, could all be utilized in this disclosure. Refined oils are similar to the unrefined oils except that they typically have undergone purification to improve one or more proper-

ties. Many such purification techniques are known to those of skill in the art such as solvent extraction, acid or base extraction, filtration, percolation, and similar purification techniques. Re-refined oils are also known as reclaimed or reprocessed oils and often are additionally processed by techniques directed to removal of spent additives and oil breakdown products.

The base oil may alternatively be described as specified in the American Petroleum Institute (API) Base Oil Interchangeability Guidelines. In other words, the base oil may be further described as one or a combination of more than one of five base oil groups: Group I (sulfur content >0.03 wt %, and/or <90 wt % saturates, viscosity index 80-120); Group II (sulfur content less than or equal to 0.03 wt %, and greater than or equal to 90 wt % saturates, viscosity index 80-120); Group III (sulfur content less than or equal to 0.03 wt %, and greater than or equal to 90 wt % saturates, viscosity index greater than or equal to 120); Group IV (all polyalphaolefins (PAO's)); and Group V (all others not included in Groups I, II, III, or IV). In one embodiment, the base oil is selected from the group consisting of API Group I, II, III, IV, V and combinations thereof. In another embodiment, the base oil is selected from the group consisting of API Group II, III, IV, and combinations thereof. In still another embodiment, the base oil is further defined as an API Group II, III, or IV oil and includes a maximum of about 49.9 wt %, typically up to a maximum of about 40 wt %, more typically up to a maximum of about 30 wt %, even more typically up to a maximum of about 20 wt %, even more typically up to a maximum of about 10 wt % and even more typically up to a maximum of about 5 wt % of the lubricating oil an API Group I or V oil. It is also contemplated that Group II and Group II basestocks prepared by hydrotreatment, hydrofinishing, hydroisomerization or other hydrogenative upgrading processes may be included in the API Group II described above. Moreover, the base oil may include Fisher Tropsch or gas to liquid GTL oils. These are disclosed for example in U.S. 2008/0076687, which is expressly incorporated herein by reference in one or more non-limiting embodiments.

The base oil is typically present in the composition in an amount of from 70 to 99.9, from 80 to 99.9, from 90 to 99.9, from 75 to 95, from 80 to 90, or from 85 to 95, parts by weight per 100 parts by weight of the composition. Alternatively, the base oil may be present in amounts of greater than 70, 75, 80, 85, 90, 91, 92, 93, 94, 95, 96, 97, 98, or 99, parts by weight per 100 parts by weight of the composition. In various embodiments, the amount of lubricating oil in a fully formulated lubricant (including diluent or carrier oils presents) is from about 80 to about 99.5 percent by weight, for example, from about 85 to about 96 percent by weight, for instance from about 90 to about 95 percent by weight. Of course, the weight percent of the base oil may be any value or range of values, both whole and fractional, within those ranges and values described above and/or may vary from the values and/or range of values above by ±5%, ±10%, ±15%, ±20%, ±25%, ±30%, etc.

#### One or More Alkylethercarboxylic Acid Corrosion Inhibitor(s):

The one or more alkylethercarboxylic acid corrosion inhibitor(s) each has the formula;



wherein R is a straight or branched chain C<sub>6</sub>-C<sub>18</sub> alkyl group and n is a number of from 0 to 5. The alkyl group may be branched or unbranched and may be further defined as, for

example, 2-ethylbutyl, n-pentyl, isopentyl, 1-methylpentyl, 1,3-dimethylbutyl, n-hexyl, 1-methylhexyl, n-heptyl, isoheptyl, 1,1,3,3-tetramethylbutyl, 1-methylheptyl, 3-methylheptyl, n-octyl, 2-ethylhexyl, 1,1,3,3-trimethylhexyl, 1,1,3,3-tetramethylpentyl, nonyl, decyl, undecyl, 1-methylundecyl, dodecyl, 1,1,3,3,5,5-hexamethylhexyl, tridecyl, tetradecyl, pentadecyl, hexadecyl, heptadecyl or octadecyl. In various embodiments, n is a number from 1 to 5, from 2 to 5, from 3 to 5, from 4 to 5, from 2 to 4, from 3 to 4, from 1 to 4, from 1 to 3, or from 1 to 2. In one embodiment, R is a mixture of C<sub>12</sub>/C<sub>14</sub> alkyl groups and n is 2.5. Alternatively, n can be further defined as having an "average" value from 1 to 5, from 2 to 5, from 3 to 5, from 4 to 5, from 2 to 4, from 3 to 4, from 1 to 4, from 1 to 3, or from 1 to 2. In these embodiments, the terminology "average value" typically refers to the mean value of n when a mixture of compounds is included. It is contemplated that, upon synthesis, a distribution of compounds may be formed such that n may be an average value. In one embodiment, a distribution of compounds includes a weight percentage majority of compounds wherein n is 3, 4, or 5 and a minority weight percentage of compounds wherein n is 0, 1, or 2. Of course, n may be any value or range of values, both whole and fractional and both actual or average (mean), within those ranges and values described above and/or may vary from the values and/or range of values above by ±5%, ±10%, ±15%, ±20%, ±25%, ±30%, etc.

In one embodiment, R is a mixture of C<sub>16</sub>/C<sub>18</sub> alkyl groups and n is 2. In still another embodiment, R is a straight or branched chain C<sub>12</sub>-C<sub>14</sub> alkyl group and n is about 3. Alternatively, R can include blends of alkyl groups that have even numbers of carbon atoms or odd numbers of carbon atoms, or both. For example, R can include mixtures of C<sub>x</sub>/C<sub>y</sub> alkyl groups wherein x and y are odd numbers or even numbers. Alternatively, one may be an odd number and the other may be an even number. Typically, x and y are numbers that differ from each other by two, e.g. 6 and 8, 8 and 10, 10 and 12, 12 and 14, 14 and 16, 16 and 18, 7 and 9, 9 and 11, 11 and 13, 13 and 15, or 15 and 17. R can also include mixtures of 3 or more alkyl groups, each of which may include even or odd numbers of carbon atoms. For example, R may include a mixture of C<sub>9</sub>, C<sub>10</sub>, C<sub>11</sub>, C<sub>12</sub>, C<sub>13</sub>, C<sub>14</sub>, and/or C<sub>15</sub> alkyl groups. Typically, if R is a mixture of alkyl groups then at least two alkylethercarboxylic acid corrosion inhibitor(s) are present. In other words, no single alkylethercarboxylic acid has two different alkyl groups represented by the same variable R. Thus, the terminology "mixture of alkyl groups" typically refers to a mixture of alkylethercarboxylic acid corrosion inhibitor(s) wherein one type of molecule has a particular alkyl group and a second or additional compounds have other types of alkyl groups.

Accordingly, it is to be understood that the terminology "one or more alkylethercarboxylic acid corrosion inhibitor(s)" may describe a single compound or a mixture of compounds, each of which are alkylethercarboxylic acid corrosion inhibitor(s) of the above described formula. The one or more alkylethercarboxylic acid corrosion inhibitor(s) act as corrosion inhibitors but are not limited to this function. Said differently, one or more alkylethercarboxylic acid corrosion inhibitor(s) may also have additional uses or functions in the composition.

Some alkylethercarboxylic acid corrosion inhibitor(s) are commercially available, for instance AKYPO RLM 25 and AKYPO RO 20 VG, from Kao Specialties Americas LLC. The alkylethercarboxylic acid corrosion inhibitor(s) may also be prepared from alcohol ethoxylates via oxidation, for instance as taught in U.S. Pat. No. 4,214,101, expressly incorporated herein by reference in one or more non-limiting

embodiments. The alkylethercarboxylic acid corrosion inhibitor(s) may also be prepared by carboxylmethylation of detergent alcohols as disclosed in U.S. Pat. No. 5,233,087 or 3,992,443, each of which is also expressly incorporated herein by reference in one or more non-limiting embodiments. It is also contemplated that the one or more alkylethercarboxylic acid corrosion inhibitor(s) may be as described in U.S. Ser. No. 61/232,060, filed on Aug. 7, 2009, the disclosure of which is expressly incorporated herein by reference in its entirety in one or more non-limiting embodiments.

The one or more alkylethercarboxylic acid corrosion inhibitor(s) are typically present in the composition in amounts of from about 0.01 to about 0.07 parts by weight per 100 parts by weight of the composition. In various embodiments, the one or more alkylethercarboxylic acid corrosion inhibitor(s) are present in amounts of about 0.01, 0.02, 0.03, 0.04, 0.05, 0.06, or 0.07, parts by weight per 100 parts by weight of the composition. In other embodiments, the one or more alkylethercarboxylic acid corrosion inhibitor(s) are present in amounts of from about 0.01 to 0.07, 0.02 to 0.06, 0.03 to 0.05, or 0.04 to 0.05, parts by weight per 100 parts by weight of the composition. In still other embodiments, the one or more alkylethercarboxylic acid corrosion inhibitor(s) may be present in amount of from 0.1 to 1 parts by weight per 100 parts by weight of the composition. In various embodiments, the one or more alkylethercarboxylic acid corrosion inhibitor(s) may be present in amounts of from 0.01 to 0.2, from 0.05 to 0.2, from 0.1 to 0.2, from 0.15 to 0.2, from 0.01 to 0.05, from 0.1 to 0.5, parts by weight per 100 parts by weight of the composition. Additional non-limiting examples of various suitable parts by weight include 0.1, 0.2, 0.3, 0.4, 0.5, 0.6, 0.7, 0.8, 0.9, and 1.0. In still other embodiments, the one or more alkylethercarboxylic acid corrosion inhibitor(s) may be present in amounts of from 0.03 to 0.07, 0.03 to 0.15, 0.03 to 0.5, 0.07 to 0.15, 0.07 to 0.5, or from 0.15 to 0.5, parts by weight per 100 parts by weight of the composition. Of course, the weight percent of the one or more alkylethercarboxylic acid corrosion inhibitor(s) may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

#### Additives:

The composition can additionally include one or more additives to improve various chemical and/or physical properties. Non-limiting examples of the one or more additives include anti-wear additives, metal passivators, rust inhibitors, viscosity index improvers, pour point depressors, dispersants, detergents, and antifriction additives. One or more of the additives may be ash-containing or ash-less as first introduced and described above. Such composition is commonly referred to as an engine oil or as an industrial oil, such as a hydraulic fluid, a turbine oil, an R&O (rust and oxidation inhibited) oil or a compressor oil.

#### Anti-Wear Additive:

The anti-wear additive first introduced above is not particularly limited and may be any known in the art. It may be ash-containing or ash-less, as first introduced and described above. In one embodiment, the anti-wear additive is selected from the group of ZDDP, zinc dialkyl-dithio phosphates, and combinations thereof. Alternatively, the anti-wear additive

may include sulfur- and/or phosphorus- and/or halogen-containing compounds, e.g. sulfurised olefins and vegetable oils, zinc dialkylthiophosphates, alkylated triphenyl phosphates, tritolyl phosphate, tricresyl phosphate, chlorinated paraffins, alkyl and aryl di- and trisulfides, amine salts of mono- and dialkyl phosphates, amine salts of methylphosphonic acid, diethanolaminomethyltolyltriazole, bis(2-ethylhexyl)aminomethyltolyltriazole, derivatives of 2,5-dimercapto-1,3,4-thiadiazole, ethyl 3-[(diisopropoxyphosphinothioyl)thio]propionate, triphenyl thiophosphate (triphenylphosphorothioate), tris(alkylphenyl)phosphorothioate and mixtures thereof (for example tris(isononylphenyl)phosphorothioate), diphenyl monononylphenyl phosphorothioate, isobutylphenyl diphenyl phosphorothioate, the dodecylamine salt of 3-hydroxy-1,3-thiaphosphetane 3-oxide, trithiophosphoric acid 5,5,5-tris(isooctyl 2-acetate], derivatives of 2-mercaptopbenzothiazole such as 1-[N,N-bis(2-ethylhexyl)aminomethyl]-2-mercaptop-1H-1,3-benzothiazole, ethoxycarbonyl-5-octylthio carbamate, and/or combinations thereof. In one embodiment, the anti-wear additive include phosphorous and sulfur, e.g. in phosphorothionates and/or dithiophosphate esters. It is also contemplated that the anti-wear additive may be as described in U.S. Ser. No. 61/232,060, filed on Aug. 7, 2009, the disclosure of which is expressly incorporated herein by reference in its entirety in one or more non-limiting embodiments.

The anti-wear additive is typically present in the composition in an amount of from 0.1 to 20, from 0.5 to 15, from 1 to 10, from 5 to 10, from 5 to 15, from 5 to 20, from 0.1 to 1, from 0.1 to 0.5, or from 0.1 to 1.5, parts by weight per 100 parts by weight of the composition. Alternatively, the anti-wear additive may be present in amounts of less than 20, less than 15, less than 10, less than 5, less than 1, less than 0.5, or less than 0.1, parts by weight per 100 parts by weight of the composition. It is also contemplated that the antiwear additive may be present in an amount of from 0.2 to 0.8, from 0.2 to 0.6, from 0.2 to 0.4, or from 0.3 to 0.5, parts by weight per 100 parts by weight of the composition. Of course, the weight percent of the anti-wear additive may be any value or range of values, both whole and fractional, within those ranges and values described above and/or may vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

#### Ashless Antiwear Additive that Includes Phosphorous:

In still other embodiments, the composition also includes an ashless antiwear additive that includes phosphorous, as first introduced above. In one embodiment, the ashless antiwear additive that includes phosphorous is further defined as a phosphate. In another embodiment, the ashless antiwear additive that includes phosphorous is further defined as a phosphite. In still another embodiment, the ashless antiwear additive that includes phosphorous is further defined as a phosphorothionate. The ashless antiwear additive that includes phosphorous may alternatively be further defined as a phosphorodithioate. In one embodiment, the ashless antiwear additive that includes phosphorous is further defined as a dithiophosphate. The ashless antiwear additive that includes phosphorous may also include an amine such as a secondary or tertiary amine. In one embodiment, the ashless antiwear additive that includes phosphorous includes an alkyl and/or dialkyl amine. Structures of suitable non-limiting examples of ashless antiwear additives that includes phosphorous are set forth immediately below:



wherein R is an alkyl group having from 1 to 10 carbon atoms.

In various embodiments, the ashless antiwear additive that includes phosphorous is typically present in the composition in an amount of from 0.01 to 20, from 0.5 to 15, from 1 to 10, from 5 to 10, from 5 to 15, from 5 to 20, from 0.1 to 1, from

0.1 to 0.5, or from 0.1 to 1.5, parts by weight per 100 parts by weight of the composition. Alternatively, the ashless antiwear additive that includes phosphorous may be present in amounts of less than 20, less than 15, less than 10, less than 5, less than 1, less than 0.5, or less than 0.1, parts by weight per

100 parts by weight of the composition. It is also contemplated that the ashless antiwear additive that includes phosphorous may be present in an amount of from 0.2 to 0.8, from 0.2 to 0.6, from 0.2 to 0.4, or from 0.3 to 0.5, parts by weight per 100 parts by weight of the composition.

Additives:

In addition to the antiwear additive(s) described above, the composition can additionally include one or more additional additives to improve various chemical and/or physical properties. Non-limiting examples of the one or more additives include antioxidants, metal passivators, viscosity index improvers, pour point depressors, dispersants, detergents, and antifriction additives. One or more of the additional additives may be ash-containing or ash-less as first introduced and described above. Such composition is commonly referred to as an engine oil or as an industrial oil, such as a hydraulic fluid, a turbine oil, an R&O (rust and oxidation inhibited) oil or a compressor oil.

Antioxidants:

Suitable, non-limiting, antioxidants include alkylated monophenols, for example 2,6-di-tert-butyl-4-methylphenol, 2-tert-butyl-4,6-dimethylphenol, 2,6-di-tert-butyl-4-ethylphenol, 2,6-di-tert-butyl-4-n-butylphenol, 2,6-di-tert-butyl-4-isobutylphenol, 2,6-dicyclopentyl-4-methylphenol, 2-( $\alpha$ -methylcyclohexyl)-4,6-dimethylphenol, 2,6-dioctadecyl-4-methylphenol, 2,4,6-tricyclohexylphenol, 2,6-di-tert-butyl-4-methoxymethylphenol, 2,6-di-nonyl-4-methylphenol, 2,4-dimethyl-6(1'-methylundec-1'-yl)phenol, 2,4-dimethyl-6(1'-methylheptadec-1'-yl)phenol, 2,4-dimethyl-6(1'-methyltridec-1'-yl)phenol, and combinations thereof.

Other non-limiting examples of suitable antioxidants includes alkylthiomethylphenols, for example 2,4-dioctylthiomethyl-6-tert-butylphenol, 2,4-dioctylthiomethyl-6-methylphenol, 2,4-dioctylthiomethyl-6-ethylphenol, 2,6-didodecylthiomethyl-4-nonylphenol, and combinations thereof. Hydroquinones and alkylated hydroquinones, for example 2,6-di-tert-butyl-4-methoxyphenol, 2,5-di-tert-butylhydroquinone, 2,5-di-tert-amylyhydroquinone, 2,6-diphenyl-4-octadecyloxyphenol, 2,6-di-tert-butylhydroquinone, 2,5-di-tert-butyl-4-hydroxyanisole, 3,5-di-tert-butyl-4-hydroxyphenylhydroxyanisole, 3,5-di-tert-butyl-4-hydroxyphenylstearate, bis-(3,5-di-tert-butyl-4-hydroxyphenyl) adipate, and combinations thereof, may also be utilized.

Furthermore, hydroxylated thiodiphenyl ethers, for example 2,2'-thiobis(6-tert-butyl-4-methylphenol), 2,2'-thiobis(4-octylphenol), 4,4'-thiobis(6-tert-butyl-3-methylphenol), 4,4'-thiobis(6-tert-butyl-2-methylphenol), 4,4'-thiobis(3,6-di-sec-amylphenol), 4,4'-bis-(2,6-dimethyl-4-hydroxyphenyl)disulfide, and combinations thereof, may also be used.

It is also contemplated that alkylidenebisphenols, for example 2,2'-methylenebis(6-tert-butyl-4-methylphenol), 2,2'-methylenebis(6-tert-butyl-4-ethylphenol), 2,2'-methylenebis[4-methyl-6-( $\alpha$ -methylcyclohexyl)phenol], 2,2'-methylenebis(4-methyl-6-cyclohexylphenol), 2,2'-methylenebis(6-nonyl-4-methylphenol), 2,2'-methylenebis(4,6-di-tert-butylphenol), 2,2'-ethylidenebis(4,6-di-tert-butylphenol), 2,2'-ethylidenebis(6-tert-butyl-4-isobutylphenol), 2,2'-methylenebis[6-( $\alpha$ -methylbenzyl)-4-nonylphenol], 2,2'-methylenebis[6-( $\alpha$ , $\alpha$ -dimethylbenzyl)-4-nonylphenol], 4,4'-methylenebis(2,6-di-tert-butylphenol), 4,4'-methylenebis(6-tert-butyl-2-methylphenol), 1,1-bis(5-tert-butyl-4-hydroxy-2-methylphenyl)butane, 2,6-bis(3-tert-butyl-5-methyl-2-hydroxybenzyl)-4-methylphenol, 1,1,3-tris(5-tert-butyl-4-hydroxy-2-methyl-phenyl) butane, 1,1-bis(5-tert-butyl-4-hydroxy-2-methyl-phenyl)-3-n-dodecylmercapto butane, ethylene glycol bis[3,3-bis(3'-tert-butyl-4'-hydroxyphenyl)

butyrate], bis(3-tert-butyl-4-hydroxy-5-methyl-phenyl)dicyclopentadiene, bis[2-(3'-tert-butyl-2'-hydroxy-5'-methylbenzyl)-6-tert-butyl-4-methylphenyl]terephthalate, 1,1-bis-(3,5-dimethyl-2-hydroxyphenyl)butane, 2,2-bis-(3,5-di-tert-butyl-4-hydroxyphenyl)propane, 2,2-bis-(5-tert-butyl-4-hydroxy-2-methylphenyl)-4-n-dodecylmercaptobutane, 1,1,5,5-tetra-(5-tert-butyl-4-hydroxy-2-methyl phenyl)pentane, and combinations thereof may be utilized as antioxidants.

O-, N- and S-benzyl compounds, for example 3,5,3',5'-tetra-tert-butyl-4,4'-dihydroxydibenzyl ether, octadecyl-4-hydroxy-3,5-dimethylbenzylmercaptoacetate, tris-(3,5-di-tert-butyl-4-hydroxybenzyl)amine, bis(4-tert-butyl-3-hydroxy-2,6-dimethylbenzyl)dithiol terephthalate, bis(3,5-di-tert-butyl-4-hydroxybenzyl)sulfide, isoctyl-3,5-di-tert-butyl-4-hydroxy benzylmercaptoacetate, and combinations thereof, may also be utilized.

Hydroxybenzylated malonates, for example dioctadecyl-2,2-bis-(3,5-di-tert-butyl-2-hydroxybenzyl)-malonate, di-octadecyl-2-(3-tert-butyl-4-hydroxy-5-methylbenzyl)-malonate, di-dodecylmercaptoethyl-2,2-bis-(3,5-di-tert-butyl-4-hydroxybenzyl)malonate, bis[4-(1,1,3,3-tetramethylbutyl)phenyl]-2,2-bis(3,5-di-tert-butyl-4-hydroxybenzyl)malonate, and combinations thereof are also suitable for use as antioxidants.

25 Triazine Compounds, for example 2,4-bis(octylmercapto)-6-(3,5-di-tert-butyl-4-hydroxyanilino)-1,3,5-triazine, 2-octylmercapto-4,6-bis(3,5-di-tert-butyl-4-hydroxyanilino)-1,3,5-triazine, 2-octylmercapto-4,6-bis(3,5-di-tert-butyl-4-hydroxyphenoxy)-1,3,5-triazine, 2,4,6-tris(3,5-di-tert-butyl-4-hydroxyphenoxy)-1,2,3-triazine, 1,3,5-tris(3,5-di-tert-butyl-4-hydroxybenzyl)isocyanurate, 1,3,5-tris(4-tert-butyl-3-hydroxy-2,6-dimethylbenzyl)2,4,6-tris(3,5-di-tert-butyl-4-hydroxyphenylethyl)-1,3,5-triazine, 1,3,5-tris(3,5-di-tert-butyl-4-hydroxyphenyl propionyl)-hexahydro-1,3,5-triazine, 1,3,5-tris(3,5-dicyclohexyl-4-hydroxybenzyl)isocyanurate, and combinations thereof, may also be used.

Additional suitable, but non-limiting examples of antioxidants include aromatic hydroxybenzyl compounds, for example 1,3,5-tris-(3,5-di-tert-butyl-4-hydroxybenzyl)-2,4,6-trimethylbenzene, 1,4-bis(3,5-di-tert-butyl-4-hydroxybenzyl)-2,3,5,6-tetramethylbenzene, 2,4,6-tris(3,5-di-tert-butyl-4-hydroxybenzyl)phenol, and combinations thereof. Benzylphosphonates, for example dimethyl-2,5-di-tert-butyl-4-hydroxybenzylphosphonate, diethyl-3,5-di-tert-butyl-4-hydroxybenzylphosphonate, dioctadecyl 3,5-di-tert-butyl-4-hydroxybenzylphosphonate, dioctadecyl-5-tert-butyl-4-hydroxy 3-methylbenzylphosphonate, the calcium salt of the monoethyl ester of 3,5-di-tert-butyl-4-hydroxybenzylphosphonic acid, and combinations thereof, may also be utilized.

50 In addition, acylaminophenols, for example 4-hydroxylauranilide, 4-hydroxystearanilide, octyl N-(3,5-di-tert-butyl-4-hydroxyphenyl)carbamate.

Esters of [3-(3,5-di-tert-butyl-4-hydroxyphenyl)propionic acid with mono- or polyhydric alcohols, e.g. with methanol, 55 ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanol, trimethylolpropane, 4-hydroxymethyl-1-phospho-2,6,7-trioxabicyclo[2.2.2]octane, and combinations thereof, may also be used. It is further contemplated that esters of  $\beta$ -(5-tert-butyl-4-hydroxy-3-methylphenyl)propionic acid with mono- or polyhydric alcohols, e.g. with methanol, ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol,

tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2, 6,7-trioxabicyclo[2.2.2]octane, and combinations thereof, may be used. Esters of  $\beta$ -(3,5-dicyclohexyl-4-hydroxyphenyl)propionic acid with mono- or polyhydric alcohols, e.g. with methanol, ethanol, octadecanol, 1,6-hexanediol, 1,9-nonenediol, ethylene glycol, 1,2-propanediol, neopentyl glycol, thiidiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane, and combinations thereof, may also be used. Moreover, esters of 3,5-di-tert-butyl-4-hydroxyphenyl acetic acid with mono- or polyhydric alcohols, e.g. with methanol, ethanol, octadecanol, 1,6-hexanediol, 1,9-nonenediol, ethylene glycol, 1,2-propanediol, neopentyl glycol, thiidiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane, and combinations thereof, may be utilized.

Additional non-limiting examples of suitable antioxidants include those that include nitrogen, such as amides of  $\beta$ -(3,5-di-tert-butyl-4-hydroxyphenyl)propionic acid e.g. N,N'-bis(3,5-di-tert-butyl-4-hydroxyphenylpropionyl)hexamethylendiamine, N,N'-bis(3,5-di-tert-butyl-4-hydroxyphenylpropionyl)trimethylenediamine, N,N'-bis(3,5-di-tert-butyl-4-hydroxyphenylpropionyl)hydrazine. Other suitable non-limiting examples of antioxidant include aminic antioxidants such as N,N'-diisopropyl-p-phenylenediamine, N,N'-di-sec-butyl-p-phenylenediamine, N,N'-bis(1,4-dimethylpentyl)-p-phenylenediamine, N,N'-bis(1-ethyl-3-methylpentyl)-p-phenylenediamine, N,N'-bis(1-methylheptyl)-p-phenylenediamine, N,N'-dicyclohexyl-p-phenylenediamine, N,N'-diphenyl-p-phenylenediamine, N,N'-bis(2-naphthyl)-p-phenylenediamine, N-isopropyl-N'-phenyl-p-phenylenediamine, N-(1,3-dimethyl-butyl)-N'-phenyl-p-phenylenediamine, N-(1-methylheptyl)-N'-phenyl-p-phenylenediamine, N-cyclohexyl-N'-phenyl-p-phenylenediamine, 4-(p-toluenesulfamoyl)diphenylamine, N,N'-dimethyl-N,N'-di-sec-butyl-p-phenylenediamine, diphenylamine, N-allyldiphenylamine, 4-isopropoxydiphenylamine, N-phenyl-1-naphthylamine, N-phenyl-2-naphthylamine, octylated diphenylamine, for example p,p'-di-tert-octyldiphenylamine, 4-n-butylaminophenol, 4-butyrylaminophenol, 4-nanoylaminophenol, 4-dodecanoylaminophenol, 4-octadecanoylaminophenol, bis(4-methoxyphenyl)amine, 2,6-di-tert-butyl-4-dimethylamino methylphenol, 2,4'-diaminodiphenylmethane, 4,4'-diaminodiphenylmethane, N,N,N',N'-tetramethyl-4,4'-diaminodiphenylmethane, 1,2-bis[(2-methyl-phenyl)amino]ethane, 1,2-bis(phenylamino)propane, (o-tolyl)biguanide, bis[4-(1',3'-dimethylbutyl)phenyl]amine, tert-octylated N-phenyl-1-naphthylamine, a mixture of mono- and dialkylated tert-butyl/tert-octyldiphenylamines, a mixture of mono- and dialkylated isopropyl/isohexyldiphenylamines, mixtures of mono- and dialkylated tert-butylidiphenylamines, 2,3-dihydro-3,3-dimethyl-4H-1,4-benzothiazine, phenothiazine, N-allylphenothiazine, N,N,N',N'-tetraphenyl-1,4-diaminobut-2-ene, N,N-bis(2,2,6,6-tetramethylpiperid-4-yl-hexamethylenediamine, bis(2,2,6,6-tetramethylpiperid-4-yl)sebacate, 2,2,6,6-tetramethylpiperidin-4-one and 2,2,6,6-tetramethylpiperidin-4-ol, and combinations thereof.

Even further non-limiting examples of suitable antioxidants includes aliphatic or aromatic phosphites, esters of thiopropanionic acid or of thiodiacetic acid, or salts of dithiocarbamic or dithiophosphoric acid, 2,2,12,12-tetramethyl-5,9-dihydroxy-3,7,1-trithiamidecane and 2,2,15,15-tetramethyl-5,12-dihydroxy-3,7,10,14-tetrathiahexadecane, and combinations thereof. Furthermore, sulfurized fatty esters, sulfurized fats and sulfurized olefins, and combinations thereof, may be used. It is also contemplated that the antioxidant may be as described in U.S. Ser. No. 61/232,060, filed on Aug. 7, 2009, the disclosure of which is expressly incorporated herein by reference in its entirety in one or more non-limiting embodiments.

The one or more antioxidants are not particularly limited in amount in the composition but are typically present in an amount of from 0.1 to 2, 0.5 to 2, 1 to 2, or 1.5 to 2, parts by weight per 100 parts by weight of the composition. Alternatively, the one or more antioxidants may be present in amounts of less than 2, less than 1.5, less than 1, or less than 0.5, parts by weight per 100 parts by weight of the composition. Of course, the weight percent of the one or more antioxidants may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

#### Metal Deactivators:

In various embodiments, one or more metal deactivators can be included in the composition. Suitable, non-limiting examples of the one or more metal deactivators include benzotriazoles and derivatives thereof, for example 4- or 5-alkylbenzotriazoles (e.g. triazole) and derivatives thereof, 4,5,6,7-tetrahydrobenzotriazole and 5,5'-methylenebisbenzotriazole; Mannich bases of benzotriazole or triazole, e.g. 1-[bis(2-ethylhexyl)aminomethyl]triazole and 1-[bis(2-ethylhexyl)aminomethyl]benzotriazole; and alkoxyalkylbenzotriazoles such as 1-(nonyloxyethyl)benzotriazole, 1-(1-butoxyethyl)benzotriazole and 1-(1-cyclohexyloxybutyl)triazole, and combinations thereof.

Additional non-limiting examples of the one or more metal deactivators include 1,2,4-triazoles and derivatives thereof, for example 3-alkyl(or aryl)-1,2,4-triazoles, and Mannich bases of 1,2,4-triazoles, such as 1-[bis(2-ethylhexyl)aminomethyl]-1,2,4-triazole; alkoxyalkyl-1,2,4-triazoles such as 1-(1-butoxyethyl)-1,2,4-triazole; and acylated 3-amino-1,2,4-triazoles, imidazole derivatives, for example 4,4'-methylenebis(2-undecyl-5-methylimidazole) and bis[(N-methyl)imidazol-2-yl]carbinol octyl ether, and combinations thereof.

Further non-limiting examples of the one or more metal deactivators include sulfur-containing heterocyclic compounds, for example 2-mercaptopbenzothiazole, 2,5-dimercapto-1,3,4-thiadiazole and derivatives thereof; and 3,5-bis[di(2-ethylhexyl)aminomethyl]-1,3,4-thiadiazolin-2-one, and combinations thereof. Even further non-limiting examples of the one or more metal deactivators include amino compounds, for example salicylidenepropylenediamine, salicylaminoguanidine and salts thereof, and combinations thereof. It is also contemplated that the metal deactivator may be as described in U.S. Ser. No. 61/232,060, filed on Aug. 7, 2009, the disclosure of which is expressly incorporated herein by reference in its entirety in one or more non-limiting embodiments.

The one or more metal deactivators are not particularly limited in amount in the composition but are typically present in an amount of from 0.01 to 0.1, from 0.05 to 0.01, or from 0.07 to 0.1, parts by weight per 100 parts by weight of the composition. Alternatively, the one or more metal deactiva-

tors may be present in amounts of less than 0.1, of less than 0.7, or less than 0.5, parts by weight per 100 parts by weight of the composition. The weight percent of the one or more metal deactivators may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Rust Inhibitors and Friction Modifiers:

In various embodiments, one or more additional rust inhibitors (in addition to the one or more alkylethercarboxylic acid corrosion inhibitor(s) described herein) and/or one or more friction modifiers can be included in the composition. Suitable, non-limiting examples of the one or more additional rust inhibitors and/or one or more friction modifiers include organic acids, their esters, metal salts, amine salts and anhydrides, for example alkyl- and alkenylsuccinic acids and their partial esters with alcohols, diols or hydroxycarboxylic acids, partial amides of alkyl- and alkenylsuccinic acids, 4-nonylphenoxyacetic acid, alkoxy- and alkoxyethoxycarboxylic acids such as dodecyloxyacetic acid, dodecyloxy(ethoxy) acetic acid and the amine salts thereof, and also N-oleoylsarcosine, sorbitan monooleate, lead naphthenate, alkenylsuccinic anhydrides, for example dodecenylysuccinic anhydride, 2-carboxymethyl-1-dodecyl-3-methylglycerol and the amine salts thereof, and combinations thereof. Additional suitable, non-limiting examples of the one or more rust inhibitors and/or friction modifiers include nitrogen-containing compounds, for example, primary, secondary or tertiary aliphatic or cycloaliphatic amines and amine salts of organic and inorganic acids, for example oil-soluble alkylammonium carboxylates, and also 1-[N,N-bis(2-hydroxyethyl)amino]-3-(4-nonylphenoxy)propan-2-ol, and combinations thereof. Further suitable, non-limiting examples include heterocyclic compounds, for example: substituted imidazolines and oxazolines, and 2-heptadecenyl-1-(2-hydroxyethyl)imidazoline, phosphorus-containing compounds, for example: Amine salts of phosphoric acid partial esters or phosphonic acid partial esters, and zinc dialkylthiophosphates, molybdenum-containing compounds, such as molybdenum dithiocarbamate and other sulfur and phosphorus containing derivatives, sulfur-containing compounds, for example: barium dinonylnaphthalenesulfonates, calcium petroleum sulfonates, alkylthio-substituted aliphatic carboxylic acids, esters of aliphatic 2-sulfocarboxylic acids and salts thereof, glycerol derivatives, for example: glycerol monooleate, 1-(alkylphenoxy)-3-(2-hydroxyethyl)glycerols, 1-(alkylphenoxy)-3-(2,3-dihydroxypropyl)glycerols and 2-carboxy-alkyl-1,3-dialkylglycerols, and combinations thereof. It is also contemplated that the rust inhibitors and friction modifiers may be as described in U.S. Ser. No. 61/232,060, filed on Aug. 7, 2009, the disclosure of which is expressly incorporated herein by reference in its entirety in one or more non-limiting embodiments.

The one or more additional rust inhibitors and/or one or more friction modifiers are not particularly limited in amount in the composition but may be present in an amount of from 0.05 to 0.5, 0.01 to 0.2, from 0.05 to 0.2, 0.1 to 0.2, 0.15 to 0.2, or 0.02 to 0.2, parts by weight per 100 parts by weight of the composition. Alternatively, the one or more additional rust inhibitors and/or one or more friction modifiers may be present in amounts of less than 0.5, less than 0.4, less than 0.3, less than 0.2, less than 0.1, less than 0.5, or less than 0.1, parts by weight per 100 parts by weight of the composition. The weight percent of the one or more rust inhibitors and friction modifiers may be any value or range of values, both whole and fractional, within those ranges and values described above

and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Viscosity Index Improvers:

In various embodiments, one or more viscosity index improvers can be included in the composition. Suitable, non-limiting examples of the one or more viscosity index improvers include polyacrylates, polymethacrylates, vinylpyrrolidone/methacrylate copolymers, polyvinylpyrrolidones, polybutenes, olefin copolymers, styrene/acrylate copolymers and polyethers, and combinations thereof. It is also contemplated that the viscosity index improvers may be as described in U.S. Ser. No. 61/232,060, filed on Aug. 7, 2009, the disclosure of which is expressly incorporated herein by reference in its entirety in one or more non-limiting embodiments. The one or more viscosity index improvers are not particularly limited in amount in the composition but are typically present in an amount of from 1 to 1, from 2 to 8, from 3 to 7, from 4 to 6, or from 4 to 5, parts by weight per 100 parts by weight of the composition. Alternatively, the one or more viscosity index improvers may be present in an amount of less than 10, 9, 8, 7, 6, 5, 4, 3, 2, or 1, part by weight per 100 parts by weight of the composition. The weight percent of the one or more viscosity index improvers may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Pour Point Depressants:

In various embodiments, one or more pour point depressants can be included in the composition. Suitable, non-limiting examples of the pour point depressants include polymethacrylate and alkylated naphthalene derivatives, and combinations thereof. It is also contemplated that the pour point depressants may be as described in U.S. Ser. No. 61/232,060, filed on Aug. 7, 2009, the disclosure of which is expressly incorporated herein by reference in its entirety in one or more non-limiting embodiments. The one or more pour point depressants are not particularly limited in amount in the composition but are typically present in an amount of from 0.1 to 1, from 0.5 to 1, or from 0.7 to 1, part by weight per 100 parts by weight of the composition. Alternatively, the one or more pour point depressants may be present in amounts of less than 1, less than 0.7, or less than 0.5, parts by weight per 100 parts by weight of the composition. The weight percent of the one or more pour point depressants may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Dispersants:

In various embodiments, one or more dispersants can be included in the composition. Suitable, non-limiting examples of the one or more dispersants include polybutenylsuccinic amides or -imides, polybutenylphosphonic acid derivatives and basic magnesium, calcium and barium sulfonates and phenolates, succinate esters and alkylphenol amines (Mannich bases), and combinations thereof. It is also contemplated that the dispersants may be as described in U.S. Ser. No. 61/232,060, filed on Aug. 7, 2009, the disclosure of which is expressly incorporated herein by reference in its entirety in one or more non-limiting embodiments.

The one or more dispersants are not particularly limited in amount in the composition but are typically present in an amount of from 0.1 to 5, from 0.5 to 4.5, from 1 to 4, from 1.5 to 3.5, from 2 to 3, or from 2.5 to 3, parts by weight per 100

parts by weight of the composition. Alternatively, the one or more dispersants may be present in an amount of less than 5, 4.5, 3.5, 3, 2.5, 2, 1.5, or 1, part by weight per 100 parts by weight of the composition. The weight percent of the one or more dispersants may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Detergents:

In various embodiments, one or more detergents can be included in the composition. Suitable, non-limiting examples of the one or more detergents include overbased or neutral metal sulphonates, phenates and salicylates, and combinations thereof. It is also contemplated that the detergents may be as described in U.S. Ser. No. 61/232,060, filed on Aug. 7, 2009, the disclosure of which is expressly incorporated herein by reference in its entirety in one or more non-limiting embodiments.

The one or more detergents are not particularly limited in amount in the composition but are typically present in an amount of from 0.1 to 5, from 0.5 to 4.5, from 1 to 4, from 1.5 to 3.5, from 2 to 3, or from 2.5 to 3, parts by weight per 100 parts by weight of the composition. Alternatively, the one or more detergents may be present in an amount of less than 5, 4.5, 3.5, 3, 2.5, 2, 1.5, or 1, part by weight per 100 parts by weight of the composition. The weight percent of the one or more detergents may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

In various embodiments, the composition is substantially free of water, e.g. includes less than 5, 4, 3, 2, or 1, weight percent of water. Alternatively, the composition may include less than 0.5 or 0.1 weight percent of water or may be free of water. Of course, the weight percent of the water may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

Additive Concentrate Package:

The instant disclosure also provides an additive concentrate package which includes one or more metal deactivators, one or more antioxidants, one or more anti-wear additives, and the one or more alkylethercarboxylic acid corrosion inhibitor(s) of this disclosure. In one embodiment, the additive concentrate package includes one or more ashless anti-wear additives including phosphorous. One or more of the additives may be ash-containing or ash-less as first introduced and described above. In various embodiments, the additive concentrate package may include one or more additional additives as described above. In one embodiment, the additive concentrate package is further defined as a hydraulic additive concentrate package. In another embodiment, the additive concentrate package includes 10-40 weight percent of an antioxidant (e.g. an aminic antioxidant, a phenolic antioxidant, or a combination of both), 0-15 weight percent of a metal deactivator (e.g. a yellow metal corrosion inhibitor), 0-15 weight percent of a corrosion inhibitor (e.g. the corrosion inhibitor of this disclosure and a ferrous metal corrosion inhibitor), 0-10 weight percent of a friction modifier (e.g. glycerol mono-oleate), 20-35 weight percent of an anti-wear additive, and 0-1 weight percent of an anti-foam additive. Additionally, 0-25 weight percent of a dispersant may also be included. Viscosity modifiers and pour point depressants may also be included but typically are not part of such packages.

The additive package may be included in the composition in amounts of from 0.1 to 1, from 0.2 to 0.9, from 0.3 to 0.8, from 0.4 to 0.7, or from 0.5 to 0.6, parts by weight per 100 parts by weight of the composition. The weight percent of the additive concentrate package may be any value or range of values, both whole and fractional, within those ranges and values described above and/or may be present in amounts that vary from the values and/or range of values above by  $\pm 5\%$ ,  $\pm 10\%$ ,  $\pm 15\%$ ,  $\pm 20\%$ ,  $\pm 25\%$ ,  $\pm 30\%$ , etc.

10 Some of the compounds described above may interact in the lubricant composition, so the components of the lubricant composition in final form may be different from those components that are initially added or combined together. Some products formed thereby, including products formed upon 15 employing the composition of this disclosure in its intended use, are not easily described or describable. Nevertheless, all such modifications, reaction products, and products formed upon employing the composition of this disclosure in its intended use, are expressly contemplated and hereby included herein. Various embodiments of this disclosure include one or more of the modification, reaction products, and products formed from employing the composition, as described above.

Method of Forming the Composition:

25 This disclosure also provides a method of forming the composition. The method includes the steps of providing the base oil, providing one or more of the alkylethercarboxylic acid corrosion inhibitor(s), and providing the antioxidant. In one embodiment, the method also includes providing the 30 ashless antiwear additive including phosphorous. The method also includes the step of combining the base oil and the one or more alkylethercarboxylic acid corrosion inhibitor(s), and optionally the ashless antiwear additive, to form the composition. The base oil, the one or more alkylethercarboxylic acid corrosion inhibitor(s), and optionally the ashless antiwear additive, may be combined in any order and each 35 individually in one or more separate parts.

Method for Reducing Corrosion of a Steel Article:

40 This disclosure also provides a method for reducing corrosion of a steel article using the composition that includes less than about 0.1 weight percent of one or more alkylethercarboxylic acid corrosion inhibitor(s). The method includes the steps of providing the base oil and providing the one or 45 more alkylethercarboxylic acid corrosion inhibitor(s). The method also includes the steps of combining the base oil and the one or more alkylethercarboxylic acid corrosion inhibitor(s) to form the composition and applying the composition to the steel article to reduce corrosion. After application of the composition to the steel article, the steel article passes corrosion testing according to ASTM D 665 B.

Method for Reducing Wear of a Metal:

50 This disclosure also provides a method for reducing wear of a metal, e.g. a metal article. The method may include any one or more of the aforementioned method steps. The method 55 of reducing wear of the metal includes the step of providing the metal and the step of applying the lubricant composition to the metal.

The step of providing the metal can occur before, after, or simultaneously with, the optional steps of providing the base oil, providing one or more of the alkylethercarboxylic acid corrosion inhibitor(s), providing the ashless antiwear additive, and/or combining the base oil, the one or more alkylethercarboxylic acid corrosion inhibitor(s), and the ashless antiwear additive to form a lubricant composition.

60 Antiwear Properties:

In various embodiments, the composition of this disclosure has improved four-ball antiwear properties. In some embodi-

ments, the method of this disclosure reduces wear of a metal, as described above, wherein the metal also has improved four-ball antiwear properties. The four-ball antiwear properties are reported as an average diameter of wear scars pursuant to ASTM D4172. The average diameter of the wear scars produced after applying the lubricant composition to the metal are at least 5% smaller than the average diameter of the wear scars produced after applying a standard to the metal. The standard includes the base oil and the antiwear additive and is free of the one or more alkylethercarboxylic acid corrosion inhibitor(s). The standard may be further described as a comparative composition that serves as a baseline against which to assess the efficacy of various embodiments of the composition of this disclosure. In various embodiments, the average diameter of the wear scars produced after applying the lubricant composition to the metal are at least 10%, 15%, 20%, 25%, 30%, 35%, 40%, 45%, 50%, 55%, 60%, etc., smaller than the average diameter of the wear scars produced after applying a standard to the metal. The metal is not particularly limited and may include steel, iron, aluminum, and the like.

In additional embodiments, the composition has improved FZG Scuffing Load Capacity measured pursuant to ASTM D5182. This scuffing test is used to determine an extent to which lubricant compositions prevent or minimized scuffing on tooth faces of gears at a lubrication gap. Scuffing typically occurs at points where gears are in mesh, e.g. at contact points where surfaces weld together briefly and are torn apart as the gears revolve, which leads to partial destruction of the surfaces. Typically, a defined load is applied to a pair of gears and the gears are engaged. After a certain period of time, the load is increased. After each engagement, and before the load is increased, the gears are visually inspected and wear is measured. If wear exceeds a certain limit, the test is terminated and the last load is documented along with an amount of material (mg) of the gears that is lost. In various embodiments, the composition has an FZG Scuffing Load Capacity of at least 10, 11, 12, or even higher, measured pursuant to ASTM D5182. Just as above, the FZG Scuffing Load Capacity may be increased 5%, 10%, 15%, etc. as compared to a standard. The standard for this evaluation may also include the base oil and the antiwear additive and be free of the one or more alkylethercarboxylic acid corrosion inhibitor(s). The standard may be further described as a comparative composition that serves as a baseline against which to assess the efficacy of the composition of this disclosure.

It is contemplated that the one or more alkylethercarboxylic acid corrosion inhibitor(s) may synergistically interact with the ashless antiwear additive to improve four-ball antiwear properties and/or scuffing load capacity. The terminology "synergistically interact" is not particularly limiting and typically describes the unexpected positive interaction of the one or more alkylethercarboxylic acid corrosion inhibitor(s) and the ashless antiwear additive. Said differently, the one or more alkylethercarboxylic acid corrosion inhibitor(s) may positively interact with the ashless antiwear additive such that unexpected improvements in corrosion inhibition and/or wear may be observed.

In one additional embodiment, the lubricant composition has improved four-ball antiwear properties and scuffing load capacity and includes the base oil, the one or more alkylethercarboxylic acid corrosion inhibitor(s), and the ashless antiwear additive including phosphorous. In this embodiment, the one or more alkylethercarboxylic acid corrosion inhibitor(s) synergistically interacts with the ashless antiwear additive to improve four-ball antiwear properties and scuffing load capacity. The average diameter of the wear scars result-

ing from the synergistic interaction in the lubricant composition of this embodiment are at least 5% smaller than the average diameter of the wear scars resulting from a standard that includes the base oil and the ashless antiwear additive and that is free of the one or more alkylethercarboxylic acid corrosion inhibitor(s), and wherein the scuffing load capacity resulting from the synergistic interaction in the lubricant composition is at least a failure load 12.

In another additional embodiment the lubricant composition has improved four-ball antiwear properties and scuffing load capacity and consists essentially of the base oil, the one or more alkylethercarboxylic acid corrosion inhibitor(s), and the ashless antiwear additive. The ashless antiwear additive may be selected from the group of phosphorothionates, phosphorodithioates, phosphates, and phosphites. In an additional embodiment, "n" of the one or more alkylethercarboxylic acid corrosion inhibitor(s) is 3 and the ashless antiwear additive is selected from the group of phosphorothionates, phosphorodithioates, phosphates, and phosphites.

Furthermore, the composition may be applied to a steel article to reduce corrosion of that article as evaluated according to ASTM D 665 B to determine whether any corrosion occurs and whether the article passes the test. The composition may also pass ASTM D 1401 with an emulsion time of less than 30, 25, 20, 15, 10, 9, 8, 7, 6, 5, or 4, minutes. Moreover, the composition may also have a calcium compatibility measured according to a filtration index of 1.5, 1.45, 1.4, 1.35, 1.3, 1.25, 1.2, 1.15, 1.1, 1.05, or 1, as determined using the modified *Lubrication Engineering method described in U.S. application Ser. No. 12/852,147*, expressly incorporated herein by reference in various non-limiting embodiments.

## EXAMPLES

### First Set of Examples

This first set of examples is entirely independent from the second set of examples set forth below.

Various alkylethercarboxylic acid corrosion inhibitors (Inhibitors 1-9) are formed according to the instant disclosure and are utilized herein. Two additional alkylethercarboxylic acid corrosion inhibitors (Inhibitors 10 and 11) are also representative examples of the corrosion inhibitor of this disclosure and are utilized herein.

Each of the Inhibitors 1-11 is used to form a lubricant composition (Compositions 1-11). Each of these Compositions is applied to a steel article to reduce corrosion of that article. The steel article is evaluated according to ASTM D 665 B to determine whether any corrosion occurs and whether the article passes the test. Each of the Inhibitors 1-11 are also used to form additional lubricant compositions (Compositions 12-22) which are evaluated to determine demulsibility according to ASTM D 1401 and calcium compatibility according to a modified method described in *Lubrication Engineering*, 2000, 56(4), pp. 22-31. In this method, a sample of the composition is treated with a calcium containing detergent to a final concentration level of 33 ppm calcium and 0.1% water in a blender for five minutes, then stored in a sealed container at 70° C. for 96 hours, then for 48 hours in the dark at room temperature. If the oil appears lucid and clear, it is filtered through a 0.8 µm filter according to AFNOR NF E 48-690, and the degree of filter blockage expressed as a filtration index according to the method is measured. A filtration index close to 1 is desired. A failure is noted if a precipitate is observed, if the filter becomes blocked during filtration, or if the filtration index greater than 2 is calculated.

Three comparative corrosion inhibitors (Comparative Inhibitors 1-3) which do not represent this disclosure are also utilized herein. These Comparative Inhibitors are used to form comparative lubricant compositions (Comparative Compositions 1-6). Comparative Compositions 1-3 are applied to a steel article to reduce corrosion of that article. The steel article is evaluated according to ASTM D 665 B to determine whether any corrosion occurs and whether the article passes the test. Comparative Compositions 4-6 are evaluated to determine demulsibility according to ASTM D 1401 and calcium compatibility according to the modified *Lubrication Engineering* method referenced above. The results of these evaluations are set forth below.

Formation of Inhibitor 1: Carboxymethylation of an Alkyl Ethoxylate

Sodium t-butoxide (3.34 g, 35.6 mmol) is dissolved in 17.5 mL of LIAL 125 at 100° C. The resulting clear and viscous solution is transferred by cannula into a mixture of sodium chloroacetate (4.11 g, 35.3 mmol) and LIAL 125 (2.5 mL, 81.1 mmol total) held at 60° C. The resulting mixture is heated to 100° C. for 20 hours, then allowed to cool to room temperature and slowly diluted with 25 mL of acetone. A white precipitate forms which is collected by filtration and washed with acetone. The filter cake is dissolved in water and the pH adjusted to below 3 with 1 M aqueous HCl. The resulting mixture is extracted 3 times with ethyl acetate and the combined organic extracts are washed with brine, dried over magnesium sulfate, filtered and concentrated to afford the carboxymethylation product of LIAL 125. The product is purified by flash chromatography. LIAL 125 is a C<sub>12</sub>-C<sub>15</sub> alkyl alcohol with a molecular weight of 207 g/m available from Sasol.

Formation of Inhibitor 2: Jones Procedure for Oxidation of Alcohol Ethoxylates

A 500 mL round bottom flask is charged with TOMADOL 23-1 (10 g) which is dissolved in 100 mL of acetone. Jones reagent is added dropwise via an addition funnel. The solution turns a dark green color. The reagent is added until an orange/red color persists. Excess Jones reagent is quenched by addition of several mL of isopropanol. Upon completion, the mixture is diluted with 100 mL of water followed by 100 mL of ethyl acetate. The organic layer is extracted, washed with 1N HCl and brine, dried over magnesium sulfate, filtered and concentrated to afford the desired ether carboxylic acid as a pale blue oil. TOMADOL 23-1 is a C<sub>12</sub>-C<sub>13</sub> alkyl 1 mol ethoxylate, Air Products.

Formation of Inhibitor 3: TEMPO/NaClO<sub>2</sub> Method for Oxidation of Alcohol Ethoxylates

A 5 L three neck round bottom flask equipped with a mechanical stirrer is charged with LUTENSOL TDA-3 (110.1 g, 0.339 mol; a C<sub>13</sub> alkyl 3 mol ethoxylate, BASF), TEMPO (3.71 g, 0.024 mol), acetonitrile (1.69 L) and 0.67 M sodium phosphate buffer (1.25 L of a 1:1 mixture of 0.67 M NaH<sub>2</sub>PO<sub>4</sub> and 0.67 M Na<sub>2</sub>HPO<sub>4</sub>). The reaction mixture is heated to 40° C. with stirring and approximately 20% of a NaClO<sub>2</sub> solution (prepared by dissolving 80% NaClO<sub>2</sub> (76.6 g, 0.68 mol) in 335 mL water) is added vial an addition funnel, followed by 20% of a bleach solution (prepared by diluting a commercial bleach (9.61 g, 0.007 mol) in 162 mL water. Commercial bleach is 5.25% NaOCl). The remaining portions of both solutions are added simultaneously over a 2 hour period.

Upon completion (about 6 to 12 hours) the reaction is cooled to room temperature and quenched with 1 L of water. The pH is adjusted by addition of NaOH followed by addition of ice cold aqueous sodium sulfite. The resulting solution is stirred for 20 minutes followed by addition of 500 mL of ethyl acetate. After stirring for 15 minutes, the organic layer is separated and discarded. An additional 200 mL of ethyl acetate is added and the solution is acidified to pH 2 with

concentrated HCl. The organic layer is separated and the aqueous layer is washed with two more portions of ethyl acetate. The organic layers are combined, washed with water, brine, dried over magnesium sulfate and concentrated. The product is a pale yellow oil.

Formation of Inhibitors 4-9:

The Inhibitors 4-9 are formed using either the Jones Method or the TEMPO method described above.

Inhibitor 4: NOVEL TDA-1, Sasol, a C<sub>13</sub> alkyl 1 mol ethoxylate, Jones Method

Inhibitor 5: NOVEL 23E1, Sasol, a C<sub>12</sub>/C<sub>13</sub> alkyl 1 mol ethoxylate, Jones Method

Inhibitor 6: AE-2, Proctor & Gamble, a C<sub>12</sub>/C<sub>14</sub> alkyl 2 mol ethoxylate, TEMPO Method

Inhibitor 7: NEODOL 23-2, Shell, a C<sub>12</sub>/C<sub>13</sub> alkyl 2 mol ethoxylate, TEMPO Method

Inhibitor 8: NEODOL 23-3, Shell, a C<sub>12</sub>/C<sub>13</sub> alkyl 3 mol ethoxylate, TEMPO Method

Inhibitor 9: TERGITOL 15-s-3, Dow, a C<sub>15</sub> alkyl 3 mol ethoxylate, TEMPO Method

Inhibitors 10 and 11:

Inhibitor 10 is a C<sub>16</sub>/C<sub>18</sub> alkyl 2 mol ethoxylate.

Inhibitor 11 is a C<sub>12</sub>/C<sub>14</sub> alkyl 2.5 mol ethoxylate.

Compositions 1-11 and Comparative Compositions 1-3:

The Compositions 1-11 are prepared using 0.05 wt % of the Inhibitors 1-11 described above, respectively, and also each include a blend of phenolic and alkylated diphenylamine antioxidants at 0.2 wt %, a triazole metal deactivator at 0.05 wt %, and a balance of a Group II base oil. Percents are weight percent based on weight of the base oil.

The Comparative Compositions 1-3 are prepared in the same way as described immediately above except that the Inhibitors 1-11 of this disclosure are replaced with one of IRGACOR L 12, MONACOR 39, and K-Corr 100. IRGACOR L 12 is an alkenyl succinic acid half ester that is commercially available from BASF. MONACOR 39 is an aspartic acid ester that is commercially available from Uniqema. K-Corr 100 is an ester/amide/carboxylate based additive that is commercially available from King Industries. After formation, each of the Compositions 1-11 and the Comparative Compositions 1-3 are evaluated using ASTM D 665 B, the results of which are set forth immediately below.

| Compositions   | Test Results<br>ASTM D 665B<br>(Pass/Fail) |
|----------------|--------------------------------------------|
| Composition 1  | Pass                                       |
| Composition 2  | Pass                                       |
| Composition 3  | Pass                                       |
| Composition 4  | Pass                                       |
| Composition 5  | Pass                                       |
| Composition 6  | Pass                                       |
| Composition 7  | Pass                                       |
| Composition 8  | Pass                                       |
| Composition 9  | Pass                                       |
| Composition 10 | Pass                                       |
| Composition 11 | Pass                                       |
| Comparative    | Pass                                       |
| Composition 1  |                                            |
| Comparative    |                                            |
| Composition 2  |                                            |
| Comparative    |                                            |
| Composition 3  | Fail<br>(Pass at 0.2%)                     |

The data set forth immediately above evidences that the Compositions 1-11 that include various alkylethercarboxylic acid corrosion inhibitors of this disclosure allow the steel article to pass ASTM D 665 B relative to corrosion. Notably, the alkylethercarboxylic acid corrosion inhibitors of this disclosure are effective at the same treat rates used with com-

23

mercially available materials IRGACOR L 12 and MONACOR 39, and at a treat rate that is lower than the treat rate used with K-Corr 100.

Compositions 12-22 and Comparative Compositions 4-6:

The Compositions 12-22 are prepared using 0.10 wt % of the Inhibitors 1-11 described above, a blend of phenolic and alkylated diphenylamine antioxidants at 0.2 wt %, a triazole metal deactivator at 0.05 wt %, and a balance of a Group II base oil. Percents are weight percent based on weight of the base oil. The Comparative Compositions 4-6 are prepared in the same way as described immediately above except that the Inhibitors of this disclosure are replaced with IRGACOR L 12, MONACOR 39, and K-Corr 100. After formation, the Compositions 12-22 and the Comparative Compositions 4-6 are tested to determine demulsibility according to ASTM D 1401 and calcium compatibility according to the modified *Lubrication Engineering* method referenced above. The results of these evaluations are set forth below.

Relative to ASTM D 1401, the time (minutes) needed for a 3 mL emulsion layer to form in each of the Compositions is measured. The volume of each of the oil, water, and emulsion phases (represented as oil/water/emulsion in the Table) is recorded in mL. The calcium compatibility is measured according to the modified *Lubrication Engineering* method referenced above. A sample of the Compositions is treated with a calcium containing detergent to a final concentration level of 33 ppm calcium and 0.1% water in a blender for five minutes, then stored in a sealed container at 70° C. for 96 hours, then for 48 hours in the dark at room temperature. If the oil appears lucid and clear, it is filtered through a 0.8 µm filter according to AFNOR NF E 48-690, and the degree of filter blockage expressed as a filtration index according to the method is measured. A filtration index close to 1 is desired. A failure is noted if a precipitate is observed, if the filter becomes blocked during filtration, or if the Filtration Index greater than 2 is calculated.

24

-continued

| Composition                  | Test Results<br>ASTM D 1401<br>(oil/water/emulsion (min)) | Calcium<br>Compatibility<br>(Filtration Index) |
|------------------------------|-----------------------------------------------------------|------------------------------------------------|
| Comparative<br>Composition 6 | 40/40/0 (8.5)                                             | 0.97                                           |

The data set forth above evidences that the various alkyl ether carboxylic acid corrosion inhibitors of this disclosure, in addition to providing to the superior results outlined above relative to ASTM D 665 B, also provide superior demulsibility and calcium compatibility. More specifically, the various alkyl ether carboxylic acid corrosion inhibitors of this disclosure allow the steel article to resist corrosion as measured using ASTM D 665 B while simultaneously avoiding issues of demulsibility and incompatibility with traces of calcium containing detergents. Accordingly, the various alkyl ether carboxylic acid corrosion inhibitors of this disclosure allow the lubricant compositions to be superior relative to corrosion resistance and at the same time resist the demulsibility and incompatibility problems that plague typical commercially available products.

Compositions 23-30 and Comparative Compositions 7-16:

Compositions 23-30 are formed according to this disclosure and include a Group II ISO VG 46 base oil, 0.48 wt % of a combination of additives described below, 0.04 wt % glycerol monooleate, and varying amounts of Inhibitor 10.

Comparative Compositions 7-16 include the same Group II ISO VG base oil, the same 0.48 wt % of the combination of additives, and the same 0.04 wt % glycerol monooleate as Compositions 23-30. However, Comparative Compositions 7-11 substitute various amounts of Irgacor NPA for Inhibitor 10. Comparative Formulations 12-16 substitute various amounts Irgacor L12 for Inhibitor 10. Irgacor NPA is a non-ylphenoxoacetic acid. Irgacor L12 is a mixture of succinic acid partial esters.

| Composition    | Test Results<br>ASTM D 1401<br>(oil/water/emulsion (min)) | Calcium<br>Compatibility<br>(Filtration Index) |
|----------------|-----------------------------------------------------------|------------------------------------------------|
| Composition 12 | 40/40/0 (6)                                               | 1.07                                           |
| Composition 13 | 40/40/0 (4)                                               | 1.36                                           |
| Composition 14 | 40/39/1 (10)                                              | 1.14                                           |
| Composition 15 | 40/40/0 (4)                                               | 1.29                                           |
| Composition 16 | 40/40/0 (7)                                               | 1.25                                           |
| Composition 17 | 40/39/1 (5)                                               | 1.22                                           |
| Composition 18 | 40/39/1 (5)                                               | 1.26                                           |
| Composition 19 | 40/40/0 (5)                                               | Not Determined                                 |
| Composition 20 | 38/39/3 (10)                                              | 1.18                                           |
| Composition 21 | 38/40/2 (30)                                              | 0.93                                           |
| Composition 22 | 40/39/1 (20)                                              | 1.06                                           |
| Comparative    | 40/40/0 (9)                                               | Fail                                           |
| Composition 4  |                                                           |                                                |
| Comparative    | 2/2/76 (30)                                               | 1.05                                           |
| Composition 5  |                                                           |                                                |

| Combination of<br>Additives | Approximate Parts by Weight Each<br>of the Additives Per 100 Parts by<br>Weight of the Combination |
|-----------------------------|----------------------------------------------------------------------------------------------------|
| Aminic                      | 51 ± 3                                                                                             |
| Antioxidant(s)              |                                                                                                    |
| EO/PO Block Copolymer(s)    | 0.4 ± 0.3                                                                                          |
| (Demulsifier)               |                                                                                                    |
| Anti-Wear Additive(s)       | 40 ± 3                                                                                             |
| Benzotriazole Derivative(s) | 8 ± 2                                                                                              |
| (Metal Deactivator)         |                                                                                                    |

Each of Compositions 23-30 and the Comparative Compositions 7-16 is applied to a steel article to reduce corrosion of that article. The steel article is evaluated according to ASTM D 665 B to determine whether any corrosion occurs and whether the article passes the test. The results of these evaluations are set forth immediately below.

|                             | Composition<br>23 | Composition<br>24 | Composition<br>25 | Composition<br>26 | Composition<br>27 |
|-----------------------------|-------------------|-------------------|-------------------|-------------------|-------------------|
| Combination<br>of Additives | 0.48              | 0.48              | 0.48              | 0.48              | 0.48              |
| Composition 10              | 0.015*            | 0.02*             | 0.025             | 0.03*             | 0.04              |
| Irgacor NPA                 | —                 | —                 | —                 | —                 | —                 |
| Irgacor L12                 | —                 | —                 | —                 | —                 | —                 |
| ASTM D 665B                 | Fail              | Pass              | Pass              | Pass              | Pass              |

\*Similar Compositions at 0.01, 0.02, and 0.03 weight percent of Composition 10 that do not include any glycerol monooleate also pass

|                          | Composition 28 | Composition 29 | Composition 30 | Comp. 7 | Comp. 8 |
|--------------------------|----------------|----------------|----------------|---------|---------|
| Combination of Additives | 0.48           | 0.48           | 0.48           | 0.48    | 0.48    |
| Composition 10           | 0.05           | 0.06           | 0.07           | —       | —       |
| Irgacor NPA              | —              | —              | —              | 0.015   | 0.02    |
| Irgacor L12              | —              | —              | —              | —       | —       |
| ASTM D 665B              | Pass           | Pass           | Pass           | Pass    | Pass    |

|                          | Comp. Composition 9 | Comp. Composition 10 | Comp. Composition 11 | Comp. Composition 12 | Comp. Composition 13 |
|--------------------------|---------------------|----------------------|----------------------|----------------------|----------------------|
| Combination of Additives | 0.48                | 0.48                 | 0.48                 | 0.48                 | 0.48                 |
| Composition 10           | —                   | —                    | —                    | —                    | —                    |
| Irgacor NPA              | 0.025               | 0.03                 | 0.07                 | —                    | —                    |
| Irgacor L12              | —                   | —                    | —                    | 0.015                | 0.02                 |
| ASTM D 665B              | Pass                | Pass                 | Pass                 | Fail                 | Fail                 |

|                          | Comp. Composition 14 | Comp. Composition 15 | Comp. Composition 16 |
|--------------------------|----------------------|----------------------|----------------------|
| Combination of Additives | 0.48                 | 0.48                 | 0.48                 |
| Composition 10           | —                    | —                    | —                    |
| Irgacor NPA              | —                    | —                    | —                    |
| Irgacor L12              | 0.025                | 0.03                 | 0.07                 |
| ASTM D 665B              | Fail                 | Fail                 | Pass                 |

| 25                       | Comp. Composition 31 | Comp. Composition 32 | Comp. Composition 33 | Comp. Composition 34 | Comp. Composition 35 |
|--------------------------|----------------------|----------------------|----------------------|----------------------|----------------------|
| Combination of Additives | 0.30                 | 0.30                 | 0.30                 | 0.30                 | 0.30                 |
| Composition 10           | 0.025                | 0.03                 | 0.05                 | 0.055                | 0.03                 |
| Irgacor L12              | —                    | —                    | —                    | —                    | —                    |
| ASTM D 665B              | Fail                 | Pass                 | Pass                 | Fail                 | Pass                 |

#### Compositions 31-37 and Comparative Compositions 17-21:

Compositions 31-34 are formed according to this disclosure and include a Group II ISO VG 46 base oil, 0.30 wt % of a combination of additives described below, and varying amounts of Inhibitor 10. Compositions 35-37 are also formed according to this disclosure and include a Group III ISO VG 46 base oil, 0.30 wt % of a combination of additives described below, and varying amounts of Inhibitor 10.

Comparative Compositions 17 and 18 include the same Group II ISO VG base oil and the same 0.30 wt % of the combination of additives as Compositions 31-34. In addition, Comparative Compositions 19-21 include the same Group III ISO VG base oil and the same 0.30 wt % of the combination of additives as Compositions 35-37. However, Comparative Compositions 17 and 18 and 19-21 substitute various amounts of Irgacor L12 for Inhibitor 10. Irgacor L12 is a mixture of succinic acid partial esters.

| 35                       | Comp. Composition 36 | Comp. Composition 37 | Comp. Composition 17 | Comp. Composition 18 |
|--------------------------|----------------------|----------------------|----------------------|----------------------|
| Combination of Additives | 0.30                 | 0.30                 | 0.30                 | 0.30                 |
| Composition 10           | 0.05                 | 0.07                 | —                    | —                    |
| Irgacor L12              | —                    | —                    | 0.03                 | 0.05                 |
| ASTM D 665B              | Pass                 | Fail                 | Fail                 | Pass                 |

| 45                       | Comp. Composition 19 | Comp. Composition 20 | Comp. Composition 21 |
|--------------------------|----------------------|----------------------|----------------------|
| Combination of Additives | 0.30                 | 0.30                 | 0.30                 |
| Composition 10           | —                    | —                    | —                    |
| Irgacor L12              | 0.03                 | 0.05                 | 0.07                 |
| ASTM D 665B              | N/A*                 | N/A*                 | N/A*                 |

| Combination of Additives    | Approximate Parts by Weight Each of the Additives Per 100 Parts by Weight of the Combination |
|-----------------------------|----------------------------------------------------------------------------------------------|
| Phenolic Antioxidant(s)     | 60 ± 5                                                                                       |
| Aminic Antioxidant(s)       | 20 ± 5                                                                                       |
| Benzotriazole Derivative(s) | 20 ± 5                                                                                       |
| (Metal Deactivator)         |                                                                                              |

Each of Compositions 31-37 and Comparative Compositions 17-21 is applied to a steel article to reduce corrosion of that article. The steel article is evaluated according to ASTM D 665 B to determine whether any corrosion occurs and whether the article passes the test. The results of these evaluations are set forth immediately below.

\*Irgacor L12 does not dissolve and thus Comparative Compositions 18-21 cannot be evaluated according to ASTM D 665B

#### Compositions 38-45 and Comparative Compositions 22-26:

Compositions 38-41 are formed according to this disclosure and include a Group II ISO VG 46 base oil, 0.40 wt % of a combination of additives described below, 0.005 wt % of glycerol monooleate, and varying amounts of Inhibitor 10. Compositions 42-45 are also formed according to this disclosure and include a Group III ISO VG 46 base oil, 0.40 wt % of a combination of additives described below, 0.005 wt % of glycerol monooleate, and varying amounts of Inhibitor 10.

Comparative Compositions 22-24 include the same Group II ISO VG base oil, the same 0.40 wt % of the combination of additives, and the same 0.005 wt % of glycerol monooleate as

Compositions 38-41. In addition, Comparative Compositions 25 and 26 include the same Group III ISO VG base oil and the same 0.40 wt % of the combination of additives, and the same 0.005 wt % of glycerol monooleate as Compositions 42-45. However, Comparative Compositions 22-26 substitute various amounts of Irgacor L12 for Inhibitor 10.

| Combination of Additives                        | Approximate Parts by Weight Each of the Additives Per 100 Parts by Weight of the Combination |
|-------------------------------------------------|----------------------------------------------------------------------------------------------|
| Phenolic Antioxidant(s)                         | 24 ± 5                                                                                       |
| Aminic Antioxidant(s)                           | 53 ± 5                                                                                       |
| Solvent(s)                                      | 15 ± 5                                                                                       |
| Benzotriazole Derivative(s) (Metal Deactivator) | 8 ± 5                                                                                        |

Each of Compositions 38-45 and Comparative Compositions 22-26 is applied to a steel article to reduce corrosion of that article. The steel article is evaluated according to ASTM D 665 B to determine whether any corrosion occurs and whether the article passes the test. The results of these evaluations are set forth immediately below.

|                          | Com-<br>position<br>38 | Com-<br>position<br>39 | Com-<br>position<br>40 | Com-<br>position<br>41 | Com-<br>position<br>42 |
|--------------------------|------------------------|------------------------|------------------------|------------------------|------------------------|
| Combination of Additives | 0.40                   | 0.40                   | 0.40                   | 0.40                   | 0.40                   |
| Composition 10           | 0.02                   | 0.03                   | 0.05                   | 0.07                   | 0.02                   |
| Irgacor L12              | —                      | —                      | —                      | —                      | —                      |
| ASTM D 665B              | Fail                   | Pass                   | Pass                   | Fail                   | Fail                   |

|                          | Com-<br>position<br>43 | Com-<br>position<br>44 | Com-<br>position<br>45 | Com-<br>position<br>22 | Com-<br>position<br>23 |
|--------------------------|------------------------|------------------------|------------------------|------------------------|------------------------|
| Combination of Additives | 0.40                   | 0.40                   | 0.40                   | 0.40                   | 0.40                   |
| Composition 10           | 0.03                   | 0.05                   | 0.07                   | —                      | —                      |
| Irgacor L12              | —                      | —                      | —                      | 0.03                   | 0.05                   |
| ASTM D 665B              | Pass                   | Fail                   | Fail                   | Fail                   | Fail                   |

|                          | Comp.<br>Composition<br>24 | Comp.<br>Composition<br>25 | Comp.<br>Composition<br>26 |
|--------------------------|----------------------------|----------------------------|----------------------------|
| Combination of Additives | 0.40                       | 0.40                       | 0.40                       |
| Composition 10           | —                          | —                          | —                          |
| Irgacor L12              | 0.07                       | 0.03                       | 0.07                       |
| ASTM D 665B              | Fail                       | Fail                       | Fail                       |

Compositions 46-53 and Comparative Compositions 27-32: Compositions 46-49 are formed according to this disclosure and include a Group II ISO VG 46 base oil, 0.48 wt % of a combination of additives described below, 0.04 wt % of glycerol monooleate, and varying amounts of Inhibitor 10. Compositions 50-53 are also formed according to this disclosure and include a Group III ISO VG 46 base oil, 0.48 wt % of a combination of additives described below, 0.04 wt % of glycerol monooleate, and varying amounts of Inhibitor 10.

Comparative Compositions 27-30 include the same Group II ISO VG base oil, the same 0.48 wt % of the combination of

additives, and the same 0.04 wt % of glycerol monooleate as Compositions 46-49. In addition, Comparative Compositions 31 and 32 include the same Group III ISO VG base oil and the same 0.48 wt % of the combination of additives, and the same 0.04 wt % of glycerol monooleate as Compositions 50-53. However, Comparative Compositions 27-32 substitute various amounts of Irgacor L12 for Inhibitor 10.

| 10 | Combination of Additives               | Approximate Parts by Weight Each of the Additives Per 100 Parts by Weight of the Combination |
|----|----------------------------------------|----------------------------------------------------------------------------------------------|
| 15 | Aminic and Phenolic Antioxidant(s)     | 75 ± 5                                                                                       |
|    | Anti-wear Additive(s)                  | 20 ± 5                                                                                       |
|    | Metal Deactivator(s)                   | 8 ± 5                                                                                        |
|    | Antifoam Additive(s)                   | 1 ± 0.5                                                                                      |
|    | EO/PO Block Copolymer(s) (Demulsifier) | 0.5 ± 0.25                                                                                   |

20 Each of Compositions 46-53 and Comparative Compositions 27-32 is applied to a steel article to reduce corrosion of that article. The steel article is evaluated according to ASTM D 665 B to determine whether any corrosion occurs and whether the article passes the test. The results of these evaluations are set forth immediately below.

| 30                       | Com-<br>position<br>46 | Com-<br>position<br>47 | Com-<br>position<br>48 | Com-<br>position<br>49 | Com-<br>position<br>50 |
|--------------------------|------------------------|------------------------|------------------------|------------------------|------------------------|
| Combination of Additives | 0.48                   | 0.48                   | 0.48                   | 0.48                   | 0.48                   |
| Composition 10           | 0.02*                  | 0.03*                  | 0.05*                  | 0.07*                  | 0.02                   |
| Irgacor L12              | —                      | —                      | —                      | —                      | —                      |
| ASTM D 665B              | Pass                   | Pass                   | Pass                   | Pass                   | Pass                   |

35 \*Similar Compositions at 0.02, 0.03, 0.05, and 0.07 weight percent of Composition 10 that do not include any glycerol monooleate also pass

| 40                       | Com-<br>position<br>51 | Com-<br>position<br>52 | Com-<br>position<br>53 | Com-<br>position<br>27 | Com-<br>position<br>28 |
|--------------------------|------------------------|------------------------|------------------------|------------------------|------------------------|
| Combination of Additives | 0.48                   | 0.48                   | 0.48                   | 0.48                   | 0.48                   |
| Composition 10           | 0.03                   | 0.05                   | 0.07                   | —                      | —                      |
| Irgacor L12              | —                      | —                      | —                      | 0.02                   | 0.03                   |
| ASTM D 665B              | Pass                   | Pass                   | Pass                   | Pass                   | Pass                   |

| 50                       | Comp.<br>Composition<br>29 | Comp.<br>Composition<br>30 | Comp.<br>Composition<br>31 | Comp.<br>Composition<br>32 |
|--------------------------|----------------------------|----------------------------|----------------------------|----------------------------|
| Combination of Additives | 0.48                       | 0.48                       | 0.48                       | 0.48                       |
| Composition 10           | —                          | —                          | —                          | —                          |
| Irgacor L12              | 0.05                       | 0.07                       | 0.02                       | 0.07                       |
| ASTM D 665B              | Pass                       | Pass                       | Pass                       | Pass                       |

60 That data set forth in the Tables above evidence that the Compositions of this disclosure that include the alkylethercarboxylic acid corrosion inhibitor allow the steel article to pass ASTM D 665 B relative to corrosion. In fact, the alkylethercarboxylic acid corrosion inhibitors of this disclosure generally perform as well, if not better, than commercially available materials and in many instances at the same or lower treat rates. In addition, the alkylethercarboxylic acid corro-

29

sion inhibitor(s) of this disclosure perform in a variety of formulations including, but not limited to, hydraulic fluids, turbine oils, R&O oils, and compressor oils.

## Second Set of Examples

This second set of examples is entirely independent from the first set of examples set forth above.

In other examples, various lubricant compositions are formed according to this disclosure. Additional comparative compositions are also formed but do not represent this disclosure.

Comparative Compositions 1A-10A do not include any corrosion inhibitor, include about 0.04 wt % of an antiwear additive (as set forth below), and a balance of Mobil Jurong VG46.

Comparative Compositions 1B-10B include about 0.03 wt % of a nonyl phenoxyacetic acid corrosion inhibitor commercially available from BASF Corporation under the trade name of Irgacor® NPA, about 0.04 wt % of an antiwear additive (as set forth below), and a balance of Mobil Jurong VG46.

Comparative Composition 1C includes about 0.03 wt % of an alkylethercarboxylic acid corrosion inhibitor, about 0.04 wt % of zinc dithiophosphate (ashed), and a balance of Mobil Jurong VG46.

Compositions 2C-10C include about 0.03 wt % of the alkylethercarboxylic acid corrosion inhibitor of this disclo-

30

sure, about 0.04 wt % of an antiwear additive (as set forth in Table 1 below), and a balance of Mobil Jurong VG46.

The alkylethercarboxylic acid corrosion inhibitor used to form Comparative Composition 1C and Compositions 5 2C-10C has a chemical structure as shown below:



After formation, the Compositions and Comparative Compositions are applied to a metal (i.e., metal bearings) and evaluated to determine four-ball antiwear properties pursuant to ASTM D4172. Each of the four-ball antiwear properties (reported as Average Diameter of Wear Scars (mm)) measured for the Compositions and Comparative Compositions are set forth in Table 1 below and illustrated in FIG. 1. In addition, a percent difference in average diameter of wear scars (mm) between (Comparative Compositions A and Compositions C), and between (Comparative Compositions B and Compositions C), and between (Comparative Compositions B and Compositions C), is also calculated and set forth in Table 1 below.

TABLE 1

| Antiwear Additive<br>(0.04 Wt %)                                   | Comparative                           |                                     |                                     | Percent Difference in Wear<br>Scar (mm) Between<br>(Comp. Compositions A and<br>Invent. Compositions C)/<br>(Comp. Compositions B and<br>Invent. Compositions C) |
|--------------------------------------------------------------------|---------------------------------------|-------------------------------------|-------------------------------------|------------------------------------------------------------------------------------------------------------------------------------------------------------------|
|                                                                    | No Corrosion<br>Inhibitor<br>0.0 Wt % | Corrosion<br>Inhibitor<br>0.03 Wt % | Corrosion<br>Inhibitor<br>0.03 Wt % |                                                                                                                                                                  |
| Zinc Dithiophosphate<br>(Ashed-Comparative)                        | 0.6 mm<br>(Comp 1A)                   | 0.85 mm<br>(Comp 1B)                | 0.95 mm<br>(Comp 1C)                | Not Applicable                                                                                                                                                   |
| Triphenyl Phosphorothionate<br>(Ashless-)                          | 1.5 mm<br>(Comp 2A)                   | 1.23 mm<br>(Comp 2B)                | 1.1 mm<br>(Invent 2C)               | -27%/-11%                                                                                                                                                        |
| Butylated Triphenyl Phosphorothionate<br>(Ashless-)                | 1.6 mm<br>(Comp 3A)                   | 1.47 mm<br>(Comp 3B)                | 0.6 mm<br>(Invent 3C)               | -63%/-59%                                                                                                                                                        |
| Nonyl Triphenyl Phosphorothionate<br>(Ashless-)                    | 1.77 mm<br>(Comp 4A)                  | 1.3 mm<br>(Comp 4B)                 | 0.61 mm<br>(Invent 4C)              | -66%/-53%                                                                                                                                                        |
| Decyl Diphenylphosphite<br>(Ashless-)                              | 1.63 mm<br>(Comp 5A)                  | 1.2 mm<br>(Comp 5B)                 | 1.1 mm<br>(Invent 5C)               | -33%/-8%                                                                                                                                                         |
| Amine Phosphate +<br>Ditridecyl Amine<br>(Ashless-)                | 1.6 mm<br>(Comp 6A)                   | 0.53 mm<br>(Comp 6B)                | 0.58 mm<br>(Invent 6C)              | -64%/+9%*                                                                                                                                                        |
| Neutral Dialkyl Dithiophosphate<br>(Ashless-)                      | 0.8 mm<br>(Comp 7A)                   | 1.6 mm<br>(Comp 7B)                 | 0.79 mm<br>(Invent 7C)              | -1%/-51%                                                                                                                                                         |
| Isopropyl Phosphorodithioate +<br>Ditridecyl Amine<br>(Ashless-)   | 0.5 mm<br>(Comp 8A)                   | 0.95 mm<br>(Comp 8B)                | 0.45 mm<br>(Invent 8C)              | -10%/-53%                                                                                                                                                        |
| Acidic Dialkyl Dithiophosphate<br>(Ashless-)                       | 0.56 mm<br>(Comp 9A)                  | 0.55 mm<br>(Comp 9B)                | 0.45 mm<br>(Invent 9C)              | 20%/-18%                                                                                                                                                         |
| Acidic Dialkyl Dithiophosphate +<br>Ditridecyl Amine<br>(Ashless-) | 0.54 mm<br>(Comp 10A)                 | 0.5 mm<br>(Comp 10B)                | 0.44 mm<br>(Invent 10C)             | -19%/-12%                                                                                                                                                        |

\*Composition 6C has larger average diameter wear scars than Comparative Composition 6B

## 31

The Comp. Corrosion Inhibitor is the Nonyl Phenoxyacetic Acid Corrosion Inhibitor described above.

The data set forth above in Table 1 shows that Compositions 2C to 10C consistently outperform Comparative Compositions 1A-10A and are associated with wear scars that have an average diameter that is about 34% smaller. In addition, the data shows that Compositions 2C to 10C outperform Comparative Compositions 1B to 5B and 7C to 10C and are associated with wear scars that have an average diameter that is about 33% smaller. This performance is both unexpected and surprising because addition of a corrosion inhibitor to a composition that includes an antiwear addition would typically be expected to cause a reduction in antiwear performance. As shown by the data in Table 1, not only is the antiwear performance not reduced but it is actually increased.

Additional lubricant compositions (Comparative Compositions 11(A-C) to 17(A-C)) are also formed as additional comparative Compositions. Comparative Compositions 11A-17A include about 0.03 wt % of Amine O corrosion inhibitor (i.e., a substituted imidazoline), about 0.04 wt % of an antiwear additive (as set forth below), and a balance of Mobil Jurong VG46.

Comparative Compositions 11B-17B include about 0.03 wt % of Irgacor® L12 corrosion inhibitor (i.e., a alkenylsuccinic acid half ester), about 0.04 wt % of an antiwear additive (as set forth below), and a balance of Mobil Jurong VG46.

Comparative Compositions 11C-17C include about 0.03 wt % of Irgacor® L17 corrosion inhibitor, about 0.04 wt % of an antiwear additive (as set forth below), and a balance of Mobil Jurong VG46.

After formation, the Comparative Compositions are applied to a metal (i.e., metal bearings) and evaluated to determine four-ball antiwear properties pursuant to ASTM D4172, as described above. These results are set forth in Table 2 below with comparisons to the Compositions set forth above.

TABLE 2

| Antiwear Additive<br>(0.04 Wt %)                                      | Corrosion<br>Inhibitor<br>0.03 Wt % | Comp.                                 | Comp.                                 | Comp.                                 | Percent Difference in<br>Wear Scar (mm)<br>Between<br>(Invent C) and<br>(Comp A)/<br>(Comp B)/(Comp C) |
|-----------------------------------------------------------------------|-------------------------------------|---------------------------------------|---------------------------------------|---------------------------------------|--------------------------------------------------------------------------------------------------------|
|                                                                       |                                     | Corrosion<br>Inhibitor 2<br>0.03 Wt % | Corrosion<br>Inhibitor 3<br>0.03 Wt % | Corrosion<br>Inhibitor 4<br>0.03 Wt % |                                                                                                        |
| Triphenyl<br>Phosphorothionate<br>(Ashless-)                          | 1.1 mm<br>(Invent 2C)               | 1.73 mm<br>(Comp 11A)                 | 1.67 mm<br>(Comp 11B)                 | 1.17 mm<br>(Comp 11C)                 | -36%/-34%/-6%                                                                                          |
| Butylated Triphenyl<br>Phosphorothionate<br>(Ashless-)                | 0.6 mm<br>(Invent 3C)               | 0.84 mm<br>(Comp 12A)                 | 1.67 mm<br>(Comp 12B)                 | 0.84 mm<br>(Comp 12C)                 | -29%/-64%/-29%                                                                                         |
| Nonyl Triphenyl<br>Phosphorothionate<br>(Ashless-)                    | 0.61 mm<br>(Invent 4C)              | 1.67 mm<br>(Comp 13A)                 | 1.27 mm<br>(Comp 13B)                 | 1.03 mm<br>(Comp 13C)                 | -63%/-52%/-41%                                                                                         |
| Amine Phosphate +<br>Ditridecyl Amine<br>(Ashless-)                   | 0.58 mm<br>(Invent 6C)              | 1.83 mm<br>(Comp 14A)                 | 1.53 mm<br>(Comp 14B)                 | 0.7 mm<br>(Comp 14C)                  | -68%/-62%/-17%                                                                                         |
| Isopropyl<br>Phosphorodithioate +<br>Ditridecyl Amine<br>(Ashless-)   | 0.45 mm<br>(Invent. 8C)             | 0.4 mm<br>(Comp 15A)                  | 0.61 mm<br>(Comp 15B)                 | 0.53 mm<br>(Comp 15C)                 | +13%*/-26%/-15%                                                                                        |
| Acidic Dialkyl<br>Dithiophosphate<br>(Ashless-)                       | 0.45 mm<br>(Invent. 9C)             | 0.54 mm<br>(Comp 16A)                 | 0.78 mm<br>(Comp 16B)                 | 1.37 mm<br>(Comp 16C)                 | -17%/-42%/-67%                                                                                         |
| Acidic Dialkyl<br>Dithiophosphate +<br>Ditridecyl Amine<br>(Ashless-) | 0.44 mm<br>(Invent. 10C)            | 0.42 mm<br>(Comp 17A)                 | 0.56 mm<br>(Comp 17B)                 | 0.69 mm<br>(Comp 17C)                 | +5%**/-21%/-36%                                                                                        |

\*Composition 8C has larger average diameter wear scars than Comparative Composition 15A

\*\*Composition 10C has larger average diameter wear scars than Comparative Composition 17A

## 32

The Comp. Corrosion Inhibitor 2 is Amine 0, commercially available from BASF Corporation.

The Comp. Corrosion Inhibitor 3 is Irgacor® L12, commercially available from BASF Corporation.

The Comp. Corrosion Inhibitor 4 is Irgacor® L17, commercially available from BASF Corporation.

Additional Examples (Examples A1/5-D1/5 and E) are also formed and evaluated to focus on the effect of the alkyl-ethercarboxylic acid corrosion inhibitor. All of these Examples include identical amounts (i.e., treat rates) of a base oil such that the identity and amounts of the base oil is a constant. The only difference between Examples is that Examples A1, B1, C1, and D1 include varying weight percentages of the alkyl-ethercarboxylic acid corrosion inhibitor described above. Examples A2, B2, C2, and D2 include varying amounts of the comparative nonyl phenoxyacetic acid corrosion inhibitor (Comp. Corr. Inhib. 1), also described above, and serve as comparative examples. Examples A3, B3, C3, and D3 include varying amounts of the comparative Amine O (Comp. Con. Inhib. 2), also described above, and also serve as comparative examples. Examples A4, B4, C4, and D4 include varying amounts of the comparative Irgacor® L12 (Comp. Con. Inhib. 3), also described above, and further serve as comparative examples. Examples A5, B5, C5, and D5 include varying amounts of the comparative Irgacor® L17 (Comp. Con. Inhib. 4), also described above, and serve as even further comparative examples. Example E includes no corrosion inhibitor whatsoever and also serves as a comparative example. These Examples are evaluated to determine four-ball antiwear properties pursuant to ASTM D4172 as a function of treat rate. The results of these evaluations are set forth in Tables 3A and B below and in FIG. 2.

TABLE 3A

|            | Invent. Corr. (wt %) | Comp. Corr. (wt %) | Comp. Inhib. 1 (wt %) | Comp. Inhib. 2 (wt %) | Comp. Inhib. 3 (wt %) | Comp. Inhib. 4 (wt %) | Avg. Diam. (mm) | Percent Difference in Wear Scar (mm) Between Invent. Corr. Inhib. (A1-D1) and Comp. Corr. Inhib. (1, 2, 3, 4) and E |
|------------|----------------------|--------------------|-----------------------|-----------------------|-----------------------|-----------------------|-----------------|---------------------------------------------------------------------------------------------------------------------|
| Example A1 | 0.03                 | —                  | —                     | —                     | —                     | —                     | 0.68            | —                                                                                                                   |
| Example A2 | —                    | 0.03               | —                     | —                     | —                     | —                     | 0.75            | -9%                                                                                                                 |
| Example A3 | —                    | —                  | 0.03                  | —                     | —                     | —                     | 0.73            | -7%                                                                                                                 |
| Example A4 | —                    | —                  | —                     | 0.03                  | —                     | —                     | 1.4             | -51%                                                                                                                |
| Example A5 | —                    | —                  | —                     | —                     | 0.03                  | 0.6                   | —               | +13%*                                                                                                               |
| Example B1 | 0.07                 | —                  | —                     | —                     | —                     | —                     | 0.60            | —                                                                                                                   |
| Example B2 | —                    | 0.07               | —                     | —                     | —                     | —                     | 0.78            | -23%                                                                                                                |
| Example B3 | —                    | —                  | 0.07                  | —                     | —                     | —                     | 1.7             | -65%                                                                                                                |
| Example B4 | —                    | —                  | —                     | 0.07                  | —                     | —                     | 1.17            | -49%                                                                                                                |
| Example B5 | —                    | —                  | —                     | —                     | 0.07                  | 0.69                  | —               | -13%                                                                                                                |
| Example C1 | 0.15                 | —                  | —                     | —                     | —                     | —                     | 0.48            | —                                                                                                                   |
| Example C2 | —                    | 0.15               | —                     | —                     | —                     | —                     | 1.13            | -58%                                                                                                                |
| Example C3 | —                    | —                  | 0.15                  | —                     | —                     | —                     | 0.64            | -25%                                                                                                                |
| Example C4 | —                    | —                  | —                     | 0.15                  | —                     | —                     | 0.65            | -26%                                                                                                                |
| Example C5 | —                    | —                  | —                     | —                     | 0.15                  | 0.66                  | —               | -27%                                                                                                                |
| Example D1 | 0.5                  | —                  | —                     | —                     | —                     | —                     | 0.46            | —                                                                                                                   |
| Example D2 | —                    | 0.5                | —                     | —                     | —                     | —                     | 0.76            | -39%                                                                                                                |
| Example D3 | —                    | —                  | 0.5                   | —                     | —                     | —                     | 1.8             | -74%                                                                                                                |
| Example D4 | —                    | —                  | —                     | 0.5                   | —                     | —                     | 0.62            | -26%                                                                                                                |
| Example D5 | —                    | —                  | —                     | —                     | 0.5                   | 0.65                  | —               | -29%                                                                                                                |
| Example E  | —                    | —                  | —                     | —                     | —                     | —                     | 0.81            | -16% (A1 to E)<br>-26% (B1 to E)<br>-41% (C1 to E)<br>-43% (D1 to E)                                                |

\*Example A1 has larger average diameter wear scars than Example A5

The data set forth in Table 3A is rearranged but identically set forth in Table 3B below such that the trends in data are more easily visualized. Table 3B includes wear scar data in mm arranged as a function of treat rate and corrosion inhibitor.

TABLE 3B

| Treat Rate of Corrosion Inhibitors | 0 wt %       | 0.03 wt %    | 0.07 wt %    | 0.15 wt %    | 0.5 wt % |
|------------------------------------|--------------|--------------|--------------|--------------|----------|
| Invent. Corr. Inhib. (E)           | 0.81 mm (A1) | 0.68 mm (B1) | 0.6 mm (C1)  | 0.48 mm (D1) | 0.46 mm  |
| Comp. Corr. Inhib. 1 (E)           | 0.81 mm (A2) | 0.75 mm (B2) | 0.78 mm (C2) | 1.13 mm (D2) | 0.76 mm  |
| Comp. Corr. Inhib. 2 (E)           | 0.81 mm (A3) | 0.73 mm (B3) | 1.7 mm (C3)  | 0.64 mm (D3) | 1.8 mm   |
| Comp. Corr. Inhib. 3 (E)           | 0.81 mm (A4) | 1.4 mm (B4)  | 1.17 mm (C4) | 0.65 mm (D4) | 0.62 mm  |
| Comp. Corr. Inhib. 4 (E)           | 0.81 mm (A5) | 0.6 mm (B5)  | 0.69 mm (C5) | 0.66 mm (D5) | 0.65 mm  |

The Invent. Con. Inhib. in Tables 3A and 3B is the alkyl ethercarboxylic acid corrosion inhibitor described above.

The Comp. Con. Inhib. 1 in Tables 3A and 3B is the Nonyl Phenoxyacetic Acid Corrosion Inhibitor described above.

The Comp. Con. Inhib. 2 in Tables 3A and 3B is Amine 0, commercially available from BASF Corporation.

The Comp. Con. Inhib. 3 in Tables 3A and 3B is Irgacor® L12, commercially available from BASF Corporation.

The Comp. Con. Inhib. 4 in Tables 3A and 3B is Irgacor® L17, commercially available from BASF Corporation.

The data set forth in Tables 3A and 3B and FIG. 2 show that the Examples A1, B1, C1, and D1, each of which include the alkyl ethercarboxylic acid corrosion inhibitor, clearly outperform Examples A(2-5) to D(2-5) and E, except that Example A1 has larger average diameter wear scars than Example A5. This overall performance is both unexpected and surprising

because the alkyl ethercarboxylic acid corrosion inhibitor consistently reduces wear wherein the comparative nonyl phenoxyacetic acid corrosion inhibitor actually increases wear in many Examples and only minimally decreases wear in others.

An additional Composition (Composition 11) and two additional Comparative Compositions (Comparative Compositions 18 and 19) are also formed. Composition 11 and Comparative Compositions 18 and 19 include identical amounts of a base oil, antioxidants, metal deactivators, friction modifiers, and anti-foam additives such that the identities and amounts of each of these components are constants. The only difference between Compositions is that Composition 11 includes 300 ppm of the alkyl ethercarboxylic acid corrosion inhibitor described above, Comparative Composition 18 includes 300 ppm of the comparative nonyl phenoxyacetic acid corrosion inhibitor, also described above, and Comparative Composition 19 includes no corrosion inhibitor whatsoever. Each of these Compositions is evaluated to determine FZG Scuffing Load Capacity of Oils pursuant to ASTM D5182. The results of these evaluations are set forth immediately below in Table 4.

TABLE 4

|                        | Comparative Example 11 | Comparative Composition 18 | Comparative Composition 19 |
|------------------------|------------------------|----------------------------|----------------------------|
| Failure Load Stage     | 12                     | 9                          | 11                         |
| Total Weight Loss (mg) | 1,143 mg               | 293 mg                     | 1,143 mg                   |

The data set forth in Table 4 indicates that Composition 11 exhibits a higher FZG Scuffing Load Capacity measured pursuant to ASTM D5182 than Comparative Composition 18. The Composition can withstand a load of stage 12 before excessive wear is observed while the Comparative Composition can only withstand a load of stage 9 (i.e., a lesser load).

This comparison of data shows that this disclosure provides special and unexpected results associated with unexpectedly high load stage.

Moreover, Comparative Composition 19 exhibits almost identical FZG properties to Example 11. Since Comparative Composition 18 includes a corrosion inhibitor and Comparative 19 does not, the data associated with Comparative Composition 19 is indicative of the typical and expected result of combining antiwear additives and corrosion inhibitors, i.e., that a decrease in antiwear properties will result due to the antagonistic relationship between the antiwear additive and the corrosion inhibitor. The instant composition not only reduces this antagonism but surprisingly reverses this negative interaction and shows synergistic results of increased wear resistance.

It is to be understood that the appended claims are not limited to express and particular compounds, compositions, or methods described in the detailed description, which may vary between particular embodiments which fall within the scope of the appended claims. With respect to any Markush groups relied upon herein for describing particular features or aspects of various embodiments, it is to be appreciated that different, special, and/or unexpected results may be obtained from each member of the respective Markush group independent from all other Markush members. Each member of a Markush group may be relied upon individually and/or in combination and provides adequate support for specific embodiments within the scope of the appended claims.

It is also to be understood that any ranges and subranges relied upon in describing various embodiments of the present disclosure independently and collectively fall within the scope of the appended claims, and are understood to describe and contemplate all ranges including whole and/or fractional values therein, even if such values are not expressly written herein. One of skill in the art readily recognizes that the enumerated ranges and subranges sufficiently describe and enable various embodiments of the present disclosure, and such ranges and subranges may be further delineated into relevant halves, thirds, quarters, fifths, and so on. As just one example, a range "of from 0.1 to 0.9" may be further delineated into a lower third, i.e., from 0.1 to 0.3, a middle third, i.e., from 0.4 to 0.6, and an upper third, i.e., from 0.7 to 0.9, which individually and collectively are within the scope of the appended claims, and may be relied upon individually and/or collectively and provide adequate support for specific embodiments within the scope of the appended claims. In addition, with respect to the language which defines or modifies a range, such as "at least," "greater than," "less than," "no more than," and the like, it is to be understood that such language includes subranges and/or an upper or lower limit. As another example, a range of "at least 10" inherently includes a subrange of from at least 10 to 35, a subrange of from at least 10 to 25, a subrange of from 25 to 35, and so on, and each subrange may be relied upon individually and/or collectively and provides adequate support for specific embodiments within the scope of the appended claims. Finally, an individual number within a disclosed range may be relied upon and provides adequate support for specific embodiments within the scope of the appended claims. For example, a range "of from 1 to 9" includes various individual integers, such as 3, as well as individual numbers including a decimal point (or fraction), such as 4.1, which may be relied upon and provide adequate support for specific embodiments within the scope of the appended claims.

The disclosure has been described in an illustrative manner, and it is to be understood that the terminology which has been used is intended to be in the nature of words of description rather than of limitation. Many modifications and variations of the present disclosure are possible in light of the

above teachings, and the disclosure may be practiced otherwise than as specifically described.

What is claimed is:

1. A lubricant composition that is substantially free of water and comprises:  
a base oil present in an amount of greater than 85 parts by weight per 100 parts by weight of said lubricant composition;  
an antioxidant; and  
one or more alkylethercarboxylic acid corrosion inhibitor(s) present in an amount of from 0.01 to 1 weight percent based on a total weight of said lubricant composition and having the formula;



wherein R is a straight or branched chain C<sub>6</sub>-C<sub>18</sub> alkyl group and n is a number of from 0 to 5.

2. A lubricant composition as set forth in claim 1 wherein said one or more alkylethercarboxylic acid corrosion inhibitor(s) are present in an amount of from 0.01 to 0.1 weight percent based on a total weight of said lubricant composition.

3. A lubricant composition as set forth in claim 1 that comprises less than 1 weight percent of water.

4. A lubricant composition as set forth in claim 1 wherein R is a straight or branched chain C<sub>12</sub>-C<sub>14</sub> alkyl group.

5. A lubricant composition as set forth in claim 1 wherein said one or more alkylethercarboxylic acid corrosion inhibitor(s) are present in an amount of from about 0.01 to about 0.07 weight percent based on a total weight of said lubricant composition.

6. A lubricant composition as set forth in claim 1 wherein said one or more alkylethercarboxylic acid corrosion inhibitor(s) are present in an amount of from about 0.02 to less than about 0.07 weight percent based on a total weight of said lubricant composition.

7. A lubricant composition as set forth in claim 1 wherein said one or more alkylethercarboxylic acid corrosion inhibitor(s) have the formula:



wherein R comprises a mixture of C<sub>12</sub> and C<sub>14</sub> alkyl groups; or

wherein R comprises a mixture of C<sub>16</sub> and C<sub>18</sub> alkyl groups.

8. A lubricant composition as set forth in claim 1 further comprising an anti-wear additive.

9. A lubricant composition as set forth in claim 8 wherein said anti-wear additive comprises phosphorous and/or sulfur.

10. A lubricant composition as set forth in claim 1 further comprising a detergent comprising calcium.

11. A lubricant composition as set forth in claim 1 wherein said base oil is further defined as an API Group I, Group II or Group III oil.

12. A lubricant composition as set forth in claim 1 wherein said base oil is further defined as a mineral or synthetic base oil or a mixture of a mineral and a synthetic base oil.

13. A lubricant composition as set forth in claim 1 that reduces corrosion of a steel article such that the steel article passes corrosion testing according to ASTM D 665 B.

37

**14.** A lubricant composition as set forth in claim **1** wherein said base oil is further defined as an API Group II oil and said one or more alkylethercarboxylic acid corrosion inhibitor(s) are present in an amount of from 0.02 to 0.07 weight percent based on a total weight of said lubricant composition, wherein said lubricant composition further comprises an anti-wear component comprising phosphorous and/or sulfur, an alkoxylated block copolymeric demulsifier, and a benzotriazole metal deactivator, and wherein said antioxidant is further defined as two aminic antioxidants.

**15.** A lubricant composition as set forth in claim **1** wherein said base oil is further defined as an API Group II oil and said one or more alkylethercarboxylic acid corrosion inhibitor(s) are present in an amount of from 0.02 to 0.07 weight percent based on a total weight of said lubricant composition, wherein said lubricant composition further comprises a benzotriazole metal deactivator, and wherein said antioxidant is further defined as an aminic antioxidant and a phenolic antioxidant.

**16.** A lubricant composition as set forth in claim **1** wherein said base oil is further defined as an API Group II oil and said one or more alkylethercarboxylic acid corrosion inhibitor(s) are present in an amount of from 0.02 to 0.07 weight percent based on a total weight of said lubricant composition, wherein said lubricant composition further comprises a benzotriazole metal deactivator, and wherein said antioxidant is further defined as two aminic antioxidants and a phenolic antioxidant.

**17.** A lubricant composition as set forth in claim **1** having improved four-ball antiwear properties and further comprising an ashless antiwear additive comprising phosphorous, wherein the four-ball antiwear properties are reported as an average diameter of wear scars pursuant to ASTM D417, wherein the average diameter of the wear scars are at least 5% smaller than the average diameter of the wear scars resulting from a standard that comprises said base oil and said ashless antiwear additive and that is free of said one or more alkylethercarboxylic acid corrosion inhibitor(s).

**18.** A lubricant composition that is substantially free of water and comprises:

a base oil present in an amount of greater than 85 parts by weight per 100 parts by weight of said lubricant composition;

an antioxidant comprising an aminic antioxidant and/or a phenolic antioxidant;

one or more alkylethercarboxylic acid corrosion inhibitor(s) present in an amount of from 0.02 to 0.05 weight percent based on a total weight of said lubricant composition and having the formula;



wherein R is a straight or branched chain C<sub>6</sub>-C<sub>18</sub> alkyl group and n is a number of from 0 to 5; and

10

5

15

20

25

30

35

40

45

50

38

an anti-wear additive comprising phosphorous and/or sulfur.

**19.** A method of reducing corrosion of a steel article, said method comprising the steps of:

A. providing a base oil;

B. providing one or more alkylethercarboxylic acid corrosion inhibitor(s) having the formula;



wherein R is a straight or branched chain C<sub>6</sub>-C<sub>18</sub> alkyl group and n is a number of from 0 to 5;

C. providing an antioxidant;

D. combining the base oil, the one or more alkylethercarboxylic acid corrosion inhibitor(s), and the antioxidant to form a composition that is substantially free of water and comprises;

the base oil present in an amount of greater than 85 parts by weight per 100 parts by weight of the lubricant composition;

the antioxidant; and

the one or more alkylethercarboxylic acid corrosion inhibitor(s) present in an amount of from 0.01 to 1 weight percent based on a total weight of the lubricant composition; and

E. applying the lubricant composition to the steel article; wherein the steel article passes corrosion testing according to ASTM D 665 B.

**20.** A method as set forth in claim **19** further comprising the step of providing an ashless antiwear additive comprising phosphorous such that said step of combining is further defined as combining the base oil, the one or more alkylethercarboxylic acid corrosion inhibitor(s), the antioxidant, and the ashless antiwear additive comprising phosphorous to form the lubricant composition further comprising the ashless antiwear additive comprising phosphorous and having improved four-ball antiwear properties,

wherein the four-ball antiwear properties are reported as an average diameter of wear scars pursuant to ASTM D417, and

wherein the average diameter of the wear scars are at least 5% smaller than the average diameter of the wear scars resulting from a standard that comprises the base oil and the ashless antiwear additive and that is free of the one or more alkylethercarboxylic acid corrosion inhibitor(s).

\* \* \* \* \*